



US006416864B1

(12) **United States Patent**  
Hayashi et al.

(10) **Patent No.:** US 6,416,864 B1  
(45) **Date of Patent:** Jul. 9, 2002

(54) **BLACK MAGNETIC COMPOSITE PARTICLES FOR A BLACK MAGNETIC TONER**

5,648,170 A \* 7/1997 Okano et al. .... 428/403  
5,922,464 A \* 7/1999 Hayashi et al. .... 428/403  
6,294,242 B1 \* 9/2001 Hayashi et al. .... 428/141

(75) Inventors: **Kazuyuki Hayashi; Hiroko Morii**,  
both of Hiroshima; **Yasuyuki Tanaka**,  
Onoda; **Seiji Ishitani**, Hiroshima, all of  
(JP)

FOREIGN PATENT DOCUMENTS

|    |            |        |
|----|------------|--------|
| EP | 0373426 A2 | 6/1990 |
| EP | 0439367 A2 | 7/1991 |
| EP | 0913431 A2 | 5/1999 |

\* cited by examiner

*Primary Examiner*—Hoa T. Le

(74) *Attorney, Agent, or Firm*—Nixon & Vanderhye P.C.

(73) Assignee: **Toda Kogyo Corporation**,  
Hiroshima-ken (JP)

(57) **ABSTRACT**

(\*) Notice: Subject to any disclaimer, the term of this patent is extended or adjusted under 35 U.S.C. 154(b) by 0 days.

Black magnetic toner comprising:  
a binder resin, and  
black magnetic composite particles comprising:  
magnetic iron oxide particles having an average particle diameter of 0.055 to 0.95  $\mu\text{m}$ ;  
a coating layer formed on the surface of said magnetic iron oxide particles, comprising at least one organo-silicon compound selected from the group consisting of:  
(1) organosilane compounds obtainable from alkoxy-silane compounds,  
(2) polysiloxanes or modified polysiloxanes, and  
(3) fluoroalkyl organosilane compounds obtainable from fluoroalkylsilane compounds; and  
a carbon black coat formed on said coating layer comprising said organosilicon compound, in an amount of 1 to 25 parts by weight based on 100 parts by weight of said magnetic iron oxide particles.

(21) Appl. No.: **09/541,725**

(22) Filed: **Apr. 3, 2000**

**Related U.S. Application Data**

(63) Continuation-in-part of application No. 09/248,283, filed on Feb. 11, 1999, now abandoned.

(30) **Foreign Application Priority Data**

Feb. 17, 1998 (JP) .... 10-52826

(51) **Int. Cl. 7** .... B32B 5/16

(52) **U.S. Cl.** .... 428/403; 428/694 BA;  
428/407; 428/900

(58) **Field of Search** .... 428/403, 694 BA,  
428/900, 407

(56) **References Cited**

**U.S. PATENT DOCUMENTS**

|               |         |                          |
|---------------|---------|--------------------------|
| 4,620,987 A   | 11/1986 | Yamashita et al.         |
| 4,937,157 A   | 6/1990  | Haack et al.             |
| 5,364,720 A   | 11/1994 | Nakazawa et al.          |
| 5,599,627 A * | 2/1997  | Aoki et al. .... 428/403 |

Such a black magnetic toner can be free from being deteriorated in electric resistance due to the existence of the carbon black coat, and as a result, is suitable as a high-resistance or insulated magnetic toner.

**16 Claims, 2 Drawing Sheets**



(X 2000)

**FIG.1**



( $\times 20000$ )

**FIG.2**



( $\times 20000$ )

**FIG.3** $(\times 20000)$ **FIG.4** $(\times 20000)$

**BLACK MAGNETIC COMPOSITE  
PARTICLES FOR A BLACK MAGNETIC  
TONER**

**CROSS REFERENCE TO RELATED  
APPLICATION**

This is a continuation-in-part of application, Ser. No. 09/248,283 filed Feb. 11, 1999, now abandoned.

**BACKGROUND OF THE INVENTION**

The present invention relates to a black magnetic toner, and more particularly, to black a black magnetic toner using magnetic composite particles, which is not only excellent in fluidity and blackness, but also small in reduction of electric resistance and, therefore, can realize a high image quality and a high copying speed, and black magnetic composite particles which not only show an excellent dispersibility in a binder resin due to less amount of carbon black fallen-off from the surface of each particle, but also have an excellent fluidity and blackness.

As one of conventional electrostatic latent image-developing methods, there has been widely known and generally adopted a so-called one component system development method of using as a developer, a magnetic toner comprising composite particles prepared by mixing and dispersing magnetic particles such as magnetite particles in a resin, without using a carrier.

The conventional development methods of using one-component magnetic toner have been classified into CPC development methods of using a low-resistance magnetic toner, and PPC development methods of using a high-resistance magnetic toner.

In the CPC methods, the low-resistance magnetic toner used therefor has an electric conductivity, and is charged by the electrostatic induction due to electric charge of the latent images. However, since the charge induced on the magnetic toner is lost while the magnetic toner is transported from a developing zone to a transfer zone, the low-resistance magnetic toner is unsuitable for the PPC development method of using an electrostatic transfer method. In order to solve this problem, there have been developed the insulated or high-resistance magnetic toners having a volume resistivity as high as not less than  $10^{14} \Omega\text{-cm}$ .

As to the insulated or high-resistance magnetic toner, it is known that the developing characteristics thereof are affected by magnetic particles exposed to the surface of the magnetic toner, or the like.

Recently, with the high image quality such as high image density or high tone gradation, or with the high copying speed of duplicating machines, it has been strongly demanded to further enhance characteristics of the insulated or high-resistance magnetic toners as a developer, especially a fluidity thereof.

With respect to such demands, in Japanese Patent Application Laid-Open (KOKAI) No. 53-94932(1978), there has been described "these high-resistance magnetic toners are deteriorated in fluidity due to the high electric resistance, so that there arises such a problem that non-uniformity of developed images tend to be caused. Namely, although the high-resistance magnetic toners for PPC development method can maintain necessary charges required for image transfer, the magnetic toners are frictionally charged even when they are present in other steps than the transfer step, where the magnetic toners are not required to be charged, e.g., in a toner bottle or on the surface of a magnetic roll, or

also slightly charged by mechano-electrets during the production process of these magnetic toners. Therefore, the magnetic toners tend to be electrostatically agglomerated, resulting in deterioration of fluidity thereof", and "It is an another object of the present invention to provide a high-resistance magnetic toner for PPC development method which is improved in fluidity, can be prevented from causing non-uniformity of developed images, and has an excellent image definition and tone gradation, thereby obtaining high-quality copies by indirect copying methods".

In recent years, with the reduction in particle size of the insulated or high-resistance magnetic toners, it has been increasingly required to enhance the fluidity thereof.

With respect to such a fact, in "Comprehensive Data Collection for Development and Utilization of Toner Materials" published by Japan Scientific Information Co., Ltd., page 121, there has been described "With extensive development of printers such as ICP, a high image quality has been required. In particular, it has been demanded to develop high-precision or high-definition printers. In Table 1, there is shown a relationship between definitions obtained by using the respective toners. As is apparent from Table 1, the smaller the particle size of wet toners, the higher the image definition is obtained. Therefore, when a dry toner is used, in order to enhance the image definition, it is also required to reduce the particle size of the toner . . . As reports of using toners having a small particle size, it has been proposed that by using toners having a particle size of 8.5 to 11  $\mu\text{m}$ , fogs on a background can be improved and toner consumption can be reduced, and further by using polyester-based toners having a particle size of 6 to 10  $\mu\text{m}$ , an image quality, a charging stability and lifetime of the developer can be improved. However, when such toners having a small particle size are used, it has been required to solve many problems. There are problems such as improvement in productivity, sharpness of particle size distribution, improvement in fluidity, etc.". 15 20 25 30 35

Further, black magnetic toners widely used at the present time, have been required to show a high degree of blackness and a high image density for line images and solid area images on copies.

With respect to this fact, on page 272 of the above-mentioned "Comprehensive Data Collection for Development and Utilization of Toner Materials", there has been described "Powder development is characterized by a high image density. However, the high image density as well as the fog density as described hereinafter, greatly influences image characteristics obtained". 40 45

There is a close relationship between properties of the magnetic toner and those of the magnetic particles mixed and dispersed in the magnetic toner.

That is, the fluidity of the magnetic toner is largely varied depending upon surface condition of the magnetic particles exposed to the surface of the magnetic toner. Therefore, the magnetic particles themselves have been strongly required to show an excellent fluidity.

The degree of blackness and density of the magnetic toner are also largely varied depending upon the degree of blackness and density of the magnetic particles as a black pigment contained in the magnetic toner.

As the black pigment, magnetite particles have been widely used from the standpoints of magnetic properties such as saturation magnetization or coercive force, low price, color tone or the like. In addition to the magnetite particles, carbon black fine particles may be added. However, in the case where the carbon black fine particles

are used in a large amount, the electric resistance is lowered, so that it is not possible to obtain an insulated or high-resistance magnetic toner.

Hitherto, in order to enhance the fluidity of the black magnetic toner, there have been many attempts of improving the fluidity of the magnetite particles mixed and dispersed in the magnetic toner. For example, there have been proposed (1) a method of forming spherical-shaped magnetite particles (Japanese Patent Application Laid-Open (KOKAI) No. 59-64852(1984)), (2) a method of exposing a silicon compound to the surface of magnetite particles (Japanese Patent Publication (KOKOKU) No. 8-25747(1996)), or the like.

Black magnetic particles for black magnetic toner, which have not only an excellent fluidity and blackness, but also an excellent dispersibility in a binder resin, are presently strongly demanded. However, black magnetic particles capable of satisfying all of these requirements have not been obtained yet.

Namely, the above-mentioned spherical magnetite particles show a higher fluidity than those of cubic magnetite particles, octahedral magnetite particles or the like. However, the fluidity of the spherical magnetite particles is still insufficient, and further the blackness is disadvantageously low.

As to the above-mentioned magnetite particles to the surface of which the silicon compound is exposed, the fluidity thereof is also still insufficient, and the blackness thereof is also disadvantageously low.

As a result of the present inventor's earnest studies for solving the above problems, it has been found that by using as a black magnetic toner, black magnetic composite particles obtained by forming a coating layer composed of at least one organosilicon compound selected from the group consisting of (1) organosilane compounds obtainable from alkoxy silane compounds, (2) polysiloxanes or modified polysiloxanes and (3) fluoroalkyl organosilane compounds obtainable from fluoroalkylsilane compounds, on the surface of magnetic iron oxide particles having an average particle size of 0.055 to 0.95  $\mu\text{m}$ , and forming a carbon black coat on the formed coating layer such that the amount of the carbon black is 1 to 25 parts by weight based on 100 parts by weight of the said magnetic iron oxide particles, the black magnetic toner can have not only an excellent fluidity and an excellent blackness, but also can show a high-resistance or an insulating property without lowering in the electric resistance. The present invention has been attained on the basis of the finding.

#### SUMMARY OF THE INVENTION

It is an object of the present invention to provide a black magnetic toner, which is not only excellent in fluidity and blackness, but also small in reduction of electric resistance and, therefore, can realize a high image quality and a high copying speed.

It is another object of the present invention to provide black magnetic particles for black magnetic toner, which are not only excellent in fluidity and blackness, but also can show an excellent dispersibility in a binder resin.

To accomplish the aims, in a first aspect of the present invention, there is provided a black magnetic toner comprising: a binder resin, and black magnetic composite particles comprising:

magnetic iron oxide particles having an average particle diameter of 0.055 to 0.95  $\mu\text{m}$ ;

a coating layer formed on the surface of the said magnetic iron oxide particles, comprising at least one organosilicon compound selected from the group consisting of:

- (1) organosilane compounds obtainable from alkoxy silane compounds,
- (2) polysiloxanes or modified polysiloxanes, and
- (3) fluoroalkyl organosilane compounds obtainable from fluoroalkylsilane compounds; and

a carbon black coat formed on the said coating layer comprising the said organosilicon compound, in an amount of 1 to 25 parts by weight based on 100 parts by weight of the said magnetic iron oxide particles.

In a second aspect of the present invention, there is provided a black magnetic toner comprising: a binder resin, and black magnetic composite particles comprising:

magnetic iron oxide particles having an average particle diameter of 0.055 to 0.95  $\mu\text{m}$ ;

a coat formed on at least a part of the surface of the magnetic iron oxide particles, comprising at least one compound selected from the group consisting of hydroxides of aluminum, oxides of aluminum, hydroxides of silicon and oxides of silicon in an amount of 0.01 to 50% by weight, calculated as Al or  $\text{SiO}_2$ , based on the total weight of the magnetic iron oxide particles;

a coating layer formed on the coat on the surface of the said magnetic iron oxide particles, comprising at least one organosilicon compound selected from the group consisting of:

- (1) organosilane compounds obtainable from alkoxy silane compounds,
- (2) polysiloxanes or modified polysiloxanes, and
- (3) fluoroalkyl organosilane compounds obtainable from fluoroalkylsilane compounds; and

a carbon black coat formed on the said coating layer comprising the said organosilicon compound, in an amount of 1 to 25 parts by weight based on 100 parts by weight of the said magnetic iron oxide particles.

In a third aspect of the present invention, there are provided black magnetic composite particles comprising:

magnetic iron oxide particles having an average particle diameter of 0.055 to 0.95  $\mu\text{m}$ ;

a coating layer formed on the surface of the said magnetic iron oxide particles, comprising at least one organosilicon compound selected from the group consisting of:

- (1) organosilane compounds obtainable from alkoxy silane compounds,
- (2) polysiloxanes or modified polysiloxanes, and
- (3) fluoroalkyl organosilane compounds obtainable from fluoroalkylsilane compounds; and

a carbon black coat formed on the said coating layer comprising the said organosilicon compound, in an amount of 1 to 25 parts by weight based on 100 parts by weight of the said magnetic iron oxide particles.

In a fourth aspect of the present invention, there are provided black magnetic composite particles comprising:

magnetic iron oxide particles having an average particle diameter of 0.055 to 0.95  $\mu\text{m}$ ;

a coat formed on at least a part of the surface of the magnetic iron oxide particles, comprising at least one compound selected from the group consisting of hydroxides of aluminum, oxides of aluminum, hydroxides of silicon and oxides of silicon in an amount of 0.01 to 50% by weight, calculated as Al or  $\text{SiO}_2$ , based on the total weight of the magnetic iron oxide particles;

a coating formed on the coat of the surface of the said magnetic iron oxide particles, comprising at least one organosilicon compound selected from the group consisting of:

(1) organosilane compounds obtainable from alkoxy-

lane compounds,

(2) polysiloxanes or modified polysiloxanes, and

(3) fluoroalkyl organosilane compounds obtainable from fluoroalkylsilane compounds; and

a carbon black coat formed on the said coating layer comprising the said organosilicon compound, in an amount of 1 to 25 parts by weight based on 100 parts by weight of the said magnetic iron oxide particles.

In a fifth aspect of the present invention, there are provided black magnetic composite particles comprising:

maghemite particles having an average particle diameter of 0.055 to 0.95  $\mu\text{m}$ ;

a coating layer formed on the surface of the said maghemite particles, comprising at least one organosilicon compound selected from the group consisting of:

(1) organosilane compounds obtainable from alkoxy-

lane compounds,

(2) polysiloxanes or modified polysiloxanes, and

(3) fluoroalkyl organosilane compounds obtainable from fluoroalkylsilane compounds; and

a carbon black coat formed on the said coating layer comprising the said organosilicon compound, in an amount of 1 to 25 parts by weight based on 100 parts by weight of the said maghemite particles.

In a sixth aspect of the present invention, there are provided black magnetic composite particles comprising:

maghemite particles having an average particle diameter of 0.055 to 0.95  $\mu\text{m}$ ;

a coat formed on at least a part of the surface of the maghemite particles, comprising at least one compound selected from the group consisting of hydroxides of aluminum, oxides of aluminum, hydroxides of silicon and oxides of silicon in an amount of 0.01 to 50% by weight, calculated as Al or  $\text{SiO}_2$ , based on the total weight of the maghemite particles;

a coating formed on the coat of the surface of the said maghemite particles, comprising at least one organosilicon compound selected from the group consisting of:

(1) organosilane compounds obtainable from alkoxy-

lane compounds,

(2) polysiloxanes or modified polysiloxanes, and

(3) fluoroalkyl organosilane compounds obtainable from fluoroalkylsilane compounds; and

a carbon black coat formed on the said coating layer comprising the said organosilicon compound, in an amount of 1 to 25 parts by weight based on 100 parts by weight of the said maghemite particles.

In a seventh aspect of the present invention, there is provided a method of mixing a binder resin with black magnetic composite particles for production of a black magnetic toner, which black magnetic composite particles comprise:

magnetic iron oxide particles having an average particle diameter of 0.055 to 0.95  $\mu\text{m}$ ;

a coating formed on the surface of the said magnetic iron oxide particles, comprising at least one organosilicon compound selected from the group consisting of:

(1) organosilane compounds obtainable from alkoxy-

lane compounds,

(2) polysiloxanes or modified polysiloxanes, and  
(3) fluoroalkyl organosilane compounds obtainable from fluoroalkylsilane compounds; and

a carbon black coat formed on the said coating layer comprising the said organosilicon compound, in an amount of 1 to 25 parts by weight based on 100 parts by weight of the said magnetic iron oxide particles.

#### BRIEF DESCRIPTION OF THE DRAWINGS

FIG. 1 is an electron micrograph ( $\times 20,000$ ) showing a particle structure of spherical magnetite particles used in Example 1.

FIG. 2 is an electron micrograph ( $\times 20,000$ ) showing a particle structure of carbon black fine particles used in Example 1.

FIG. 3 is an electron micrograph ( $\times 20,000$ ) showing a particle structure of black magnetic composite particles obtained in Example 1.

FIG. 4 is an electron micrograph ( $\times 20,000$ ) showing a particle structure of mixed particles composed of the spherical magnetite particles and the carbon black fine particles, for comparative purpose.

#### DETAILED DESCRIPTION OF THE INVENTION

The present invention is now described in detail below.

First, the black magnetic composite particles used for the black magnetic toner according to the present invention are described.

The black magnetic composite particles according to the present invention, comprise magnetic iron oxide particles as core particles having an average particle diameter of 0.055 to 0.95  $\mu\text{m}$ , a coating comprising an organosilicon compound which is formed on the surface of each magnetic iron oxide particle, and a carbon black coat formed on the coating layer comprising the organosilicon compound.

As the magnetic iron oxide particles used as core particles in the present invention, there may be exemplified magnetite particles ( $\text{Fe}_3\text{O}_4$ ,  $0 < X \leq 1$ ), maghemite particles ( $\gamma\text{-Fe}_2\text{O}_3$ ) or a mixture of these particles.

As the magnetic iron oxide particles as core particles, from the viewpoint of a particle shape thereof, there may be exemplified isotropic particles having a ratio of an average particle length (average major diameter) to an average particle breadth (average minor diameter) of usually not less than 1.0 and less than 2.0, preferably 1.0 to 1.8, more preferably 1.0 to 1.5, such as spherical particles, granular particles or polyhedral particles, e.g., hexahedral particles or octahedral particles, or anisotropic particles having an aspect ratio (average major axial diameter/average minor axial diameter; hereinafter referred to merely as "aspect ratio") of not less than 2:1, such as acicular particles, spindle-shaped particles or rice ball-shaped particles. In the consideration of the fluidity of the obtained black magnetic composite particles, the magnetic iron oxide particles having an isotropic shape are preferred. Among them, the spherical particles are more preferred.

In the case of the isotropic magnetic iron oxide particles, the average particle size (diameter) thereof is 0.055 to 0.95  $\mu\text{m}$ , preferably 0.065 to 0.75  $\mu\text{m}$ , more preferably 0.065 to 0.45  $\mu\text{m}$ . In the case of the anisotropic magnetic iron oxide particles, the average major axial diameter thereof is 0.055 to 0.95  $\mu\text{m}$ , preferably 0.065 to 0.75  $\mu\text{m}$ , more preferably 0.065 to 0.45  $\mu\text{m}$ , and the aspect ratio (average major axial diameter/average minor axial diameter) thereof is 2:1 to 20:1, preferably 2:1 to 15:1, more preferably 2:1 to 10:1.

When the average particle size of the magnetic iron oxide particles is more than 0.95  $\mu\text{m}$ , the obtained black magnetic composite particles are coarse particles and are deteriorated in tinting strength. On the other hand, when the average particle size is less than 0.055  $\mu\text{m}$ , the intermolecular force between the particles is increased due to the reduction in particle size (fine particle), so that agglomeration of the particles tends to be caused. As a result, it becomes difficult to uniformly coat the surfaces of the magnetic iron oxide particles with the organosilicon compounds, and uniformly form the carbon black coat on the surface of the coating layer comprising the organosilicon compounds.

Further, in the case where the upper limit of the aspect ratio of the anisotropic magnetic iron oxide particles exceeds 20:1, the particles tend to be entangled with each other, and it also becomes difficult to uniformly coat the surfaces of the magnetic iron oxide particles with the organosilicon compounds, and uniformly form the carbon black coat on the surface of the coating layer composed of the organosilicon compounds.

As to the particle size distribution of the magnetic iron oxide particles, the geometrical standard deviation value thereof is preferably not more than 2.0, more preferably not more than 1.8, still more preferably not more than 1.6. When the geometrical standard deviation value thereof is more than 2.0, coarse particles are contained therein, so that the particles are inhibited from being uniformly dispersed. As a result, it also becomes difficult to uniformly coat the surfaces of the magnetic iron oxide particles with the organosilicon compounds, and uniformly form the carbon black coat on the surface of the coating layer composed of the organosilicon compounds. The lower limit of the geometrical standard deviation value is 1.01. It is industrially difficult to obtain particles having a geometrical standard deviation value of less than 1.01.

The BET specific surface area of the magnetic iron oxide particles thereof is not less than 0.5  $\text{m}^2/\text{g}$ . When the BET specific surface area is less than 0.5  $\text{m}^2/\text{g}$ , the magnetic iron oxide particles may become coarse particles, or the sintering between the particles may be caused, so that the obtained black magnetic composite particles also may become coarse particles and tend to be deteriorated in tinting strength. In the consideration of the tinting strength of the obtained black magnetic composite particles, the BET specific surface area of the magnetic iron oxide particles is preferably not less than 1.0  $\text{m}^2/\text{g}$ , more preferably 3.0  $\text{m}^2/\text{g}$ . Further, in the consideration of uniformly coating the surfaces of the magnetic iron oxide particles with the organosilicon compounds, and uniformly forming the carbon black coat on the coating layer composed of the organosilicon compounds, the upper limit of the BET specific surface area of the magnetic iron oxide particles, is usually 70  $\text{m}^2/\text{g}$ , preferably 50  $\text{m}^2/\text{g}$ , more preferably 20  $\text{m}^2/\text{g}$ .

As to the fluidity of the magnetic iron oxide particles, the fluidity index thereof is about 25 to about 44. Among the magnetic iron oxide particles having various shapes, the spherical particles are excellent in fluidity, for example, the fluidity index thereof is about 30 to about 44.

As to the blackness of the magnetic iron oxide particles, in the case of the magnetite particles, the lower limit thereof is usually 18.0 when represented by  $L^*$  value, and the upper limit thereof is usually 25.0, preferably 24.0 when represented by  $L^*$  value. In the case of maghemite particles, the lower limit thereof is usually more than 18.0 when represented by  $L^*$  value, and the upper limit thereof is usually 32, preferably 30 when represented by  $L^*$  value. When the  $L^*$

value exceeds the above-mentioned upper limit, the lightness of the particles is increased, so that it is difficult to obtain black magnetic composite particles having a sufficient blackness.

As to the magnetic properties of the magnetic iron oxide particles, the coercive force value thereof is usually about 10 to about 350 Oe, preferably 20 to about 330 Oe; the saturation magnetization value in a magnetic field of 10 kOe is usually about 50 to about 91 emu/g, preferably about 60 to about 90 emu/g; and the residual magnetization value in a magnetic field of 10 kOe is usually about 1 to about 35 emu/g, preferably about 3 to about 30 emu/g.

The particle shape and particle size of the black magnetic composite particles according to the present invention are considerably varied depending upon those of the magnetic iron oxide particles as core particles. The black magnetic composite particles have a similar particle shape to that of the magnetic iron oxide particle as core particle, and a slightly larger particle size than that of the magnetic iron oxide particles as core particles.

More specifically, when the isotropic magnetic iron oxide particles are used as core particles, the obtained black magnetic composite particles according to the present invention, have an average particle size of usually 0.06 to 1.0  $\mu\text{m}$ , preferably 0.07 to 0.8  $\mu\text{m}$ , more preferably 0.07 to 0.5  $\mu\text{m}$  and a ratio of an average particle length to an average particle breadth of usually not less than 1.0 and less than 2.0, preferably 1.0 to 1.8, more preferably 1.0 to 1.5. When the anisotropic magnetic iron oxide particles are used as core particles, the obtained black magnetic composite particles according to the present invention, have an average particle size of usually 0.06 to 1.0  $\mu\text{m}$ , preferably 0.07 to 0.8  $\mu\text{m}$ , more preferably 0.07 to 0.5  $\mu\text{m}$ .

When the average particle size of the black magnetic composite particles is more than 1.0  $\mu\text{m}$ , the obtained black magnetic composite particles may be coarse particles, and deteriorated in tinting strength. On the other hand, when the average particle size thereof is less than 0.06  $\mu\text{m}$ , the black magnetic composite particles tends to be agglomerated by the increase of intermolecular force due to the reduction in particle size, thereby deteriorating the dispersibility in a binder resin upon production of the magnetic toner.

When the anisotropic magnetic iron oxide particles are used as core particles, the upper limit of the aspect ratio of the obtained black magnetic composite particles according to the present invention, is usually 20:1, preferably 18:1, more preferably 15:1. When the aspect ratio is more than 20:1, the black magnetic composite particles may be entangled with each other in the binder resin, so that the dispersibility in binder resin tends to be deteriorated.

The geometrical standard deviation value of the black magnetic composite particles according to the present invention is preferably not more than 2.0, more preferably 1.01 to 1.8, still more preferably 1.01 to 1.6. The lower limit of the geometrical standard deviation value thereof is preferably 1.01. When the geometrical standard deviation value thereof is more than 2.0, the tinting strength of the black magnetic composite particles is likely to be deteriorated due to the existence of coarse particles therein. It is industrially difficult to obtain such particles having a geometrical standard deviation of less than 1.01.

The BET specific surface area of the black magnetic composite particles according to the present invention, is usually 1 to 200  $\text{m}^2/\text{g}$ , preferably 2 to 150  $\text{m}^2/\text{g}$ , more preferably 2.5 to 100  $\text{m}^2/\text{g}$ . When the BET specific surface area thereof is less than 1  $\text{m}^2/\text{g}$ , the obtained black magnetic

composite particles may be coarse, and the sintering between the black magnetic composite particles is caused, thereby deteriorating the tinting strength. On the other hand, when the BET specific surface area is more than 200 m<sup>2</sup>/g, the black magnetic composite particles tend to be agglomerated together by the increase in intermolecular force due to the reduction in particle size, thereby deteriorating the dispersibility in a binder resin upon production of the magnetic toner.

As to the fluidity of the black magnetic composite particles according to the present invention, the fluidity index thereof is preferably 45 to 80, more preferably 46 to 80, still more preferably 47 to 80. When the fluidity index thereof is less than 45, the fluidity of the black magnetic composite particles becomes insufficient, thereby failing to improve the fluidity of the finally obtained magnetic toner. Further, in the production process of the magnetic toner, there tend to be caused defects such as clogging of hopper, etc., thereby deteriorating the handling property or workability.

As to the blackness of the black magnetic composite particles according to the present invention, in the case magnetite particles are used as core particles, the upper limit of the blackness of the black magnetic composite particles is usually 20.0, preferably 19.0, more preferably 18.0 when represented by L\* value. In the case maghemite particles are used as core particles, the upper limit of the blackness of the black magnetic composite particles is usually 20.0, preferably 19.5, more preferably 19.0 when represented by L\* value. When the L\* value thereof is more than 20.0, the lightness of the obtained black magnetic composite particles becomes high, so that the black magnetic composite particles having a sufficient blackness cannot be obtained. The lower limit of the blackness thereof is 15 when represented by L\* value.

The dispersibility in binder resin of the black magnetic composite particles according to the present invention, is preferably 4th or 5th rank, more preferably 5th rank when evaluated by the method described hereinafter.

The percentage of desorption of carbon black from the black magnetic composite particles according to the present invention, is preferably not more than 20%, more preferably not more than 10%. When the desorption percentage of the carbon black is more than 20%, the desorbed carbon black tend to inhibit the black magnetic composite particles from being uniformly dispersed in the binder resin upon production of the magnetic toner.

The magnetic properties of the black magnetic composite particles according to the present invention, can be controlled by appropriately selecting kind and particle shape of the magnetic iron oxide particles as core particles. Similarly to magnetic properties of magnetic particles ordinarily used for the production of magnetic toner, the coercive force of the black magnetic composite particles according to the present invention, is usually about 10 to about 350 Oe, preferably about 20 to about 330 Oe; the saturation magnetization in a magnetic field of 10 kOe is usually about 50 to about 91 emu/g, preferably about 60 to about 90 emu/g; and the residual magnetization in a magnetic field of 10 kOe is usually about 1 to about 35 emu/g, preferably about 3 to about 30 emu/g.

The coating layer formed on the surfaces of the core particles comprises at least one organosilicon compound selected from the group consisting of (1) organosilane compounds obtainable from alkoxy silane compounds; (2) polysiloxanes, or modified polysiloxanes selected from the group consisting of (A) polysiloxanes modified with at least

one compound selected from the group consisting of polyethers, polyesters and epoxy compounds (hereinafter referred to merely as "modified polysiloxanes"), and (B) polysiloxanes whose molecular terminal is modified with at least one group selected from the group consisting of carboxylic acid groups, alcohol groups and a hydroxyl group; and (3) fluoroalkyl organosilane compounds obtainable from fluoroalkylsilane compounds.

The organosilane compounds (1) may be produced by 10 drying or heat-treating alkoxy silane compounds represented by the formula (I):



wherein R<sup>1</sup> is C<sub>6</sub>H<sub>5</sub>—, (CH<sub>3</sub>)<sub>2</sub>CHCH<sub>2</sub>— or n-C<sub>b</sub>H<sub>2b+1</sub>— (wherein b is an integer of 1 to 18); X is CH<sub>3</sub>O— or C<sub>2</sub>H<sub>5</sub>O—; and a is an integer of 0 to 3.

The drying or heat-treatment of the alkoxy silane compounds may be conducted, for example, at a temperature of usually 40 to 200° C., preferably 60 to 150° C. for usually 20 10 minutes to 12 hours, preferably 30 minutes to 3 hours.

Specific examples of the alkoxy silane compounds may include methyl triethoxysilane, dimethyl diethoxysilane, phenyl triethoxysilane, diphenyl diethoxysilane, methyl trimethoxysilane, dimethyl dimethoxysilane, phenyl trimethoxysilane, diphenyl dimethoxysilane, isobutyl trimethoxysilane, decyl trimethoxysilane or the like. Among these alkoxy silane compounds, in view of the desorption percentage and the adhering effect of carbon black, methyl triethoxysilane, phenyl triethoxysilane, methyl trimethoxysilane, dimethyl dimethoxysilane and isobutyl trimethoxysilane are preferred, and methyl triethoxysilane and methyl trimethoxysilane are more preferred.

As the polysiloxanes (2), there may be used those compounds represented by the formula (II):



wherein R<sup>2</sup> is H— or CH<sub>3</sub>—, and d is an integer of 15 to 450.

Among these polysiloxanes, in view of the desorption percentage and the adhering effect of carbon black, polysiloxanes having methyl hydrogen siloxane units are preferred.

As the modified polysiloxanes (2-A), there may be used: 50 (a1) polysiloxanes modified with polyethers represented by the formula (III):



wherein R<sup>3</sup> is  $-(\text{CH}_2)_h-$ ; R<sup>4</sup> is  $-(\text{CH}_2)_i-\text{CH}_3$ ; R<sup>5</sup> is  $-\text{OH}$ ,  $-\text{COOH}$ ,  $-\text{CH}=\text{CH}_2$ ,  $-\text{C}(\text{CH}_3)=\text{CH}_2$  or  $-(\text{CH}_2)_j-\text{CH}_3$ ; R<sup>6</sup> is  $-(\text{CH}_2)_k-\text{CH}_3$ ; g and h are an integer of 1 to 15; i, j and k are an integer of 0 to 15; e is an integer of 1 to 50; and f is an integer of 1 to 300;

(a2) polysiloxanes modified with polyesters represented by the formula (IV):

(IV)



wherein  $R^7$ ,  $R^8$  and  $R^9$  are  $-(CH_2)_q-$  and may be the same or different;  $R^{10}$  is  $-OH$ ,  $-COOH$ ,  $-CH=CH_2$ ,  $-C(CH_3)=CH_2$  or  $-(CH_2)_r-CH_3$ ;  $R^{11}$  is  $-(CH_2)_s-CH_3$ ;  $n$  and  $q$  are an integer of 1 to 15;  $r$  and  $s$  are an integer of 0 to 15;  $e$  is an integer of 1 to 50; and  $f$  is an integer of 1 to 300;

(a3) polysiloxanes modified with epoxy compounds represented by the formula (V):

(V)



wherein  $R^{12}$  is  $-(CH_2)_v-$ ;  $v$  is an integer of 1 to 15;  $t$  is an integer of 1 to 50; and  $u$  is an integer of 1 to 300; or a mixture thereof.

Among these modified polysiloxanes (2-A), in view of the desorption percentage and the adhering effect of carbon black, the polysiloxanes modified with the polyethers represented by the formula (III), are preferred.

As the terminal-modified polysiloxanes (2-B), there may be used those represented by the formula (VI):

(VI)



wherein  $R^{13}$  and  $R^{14}$  are  $-OH$ ,  $R^{16}OH$  or  $R^{17}COOH$  and may be the same or different;  $R^{15}$  is  $-CH_3$  or  $-C_6H_5$ ;  $R^{16}$  and  $R^{17}$  are  $-(CH_2)_y-$ ;  $y$  is an integer of 1 to 15;  $w$  is an integer of 1 to 200; and  $x$  is an integer of 0 to 100.

Among these terminal-modified polysiloxanes, in view of the desorption percentage and the adhering effect of carbon black, the polysiloxanes whose terminals are modified with carboxylic acid groups are preferred.

The fluoroalkyl organosilane compounds (3) may be produced by drying or heat-treating fluoroalkylsilane compounds represented by the formula (VII):



wherein  $R^{18}$  is  $CH_3-$ ,  $C_2H_5-$ ,  $CH_3O-$  or  $C_2H_5O-$ ;  $X$  is  $CH_3O-$  or  $C_2H_5O-$ ; and  $z$  is an integer of 0 to 15; and  $a'$  is an integer of 0 to 3.

The drying or the heat-treatment of the fluoroalkylsilane compounds may be conducted, for example, at a temperature of usually 40 to 200° C., preferably 60 to 150° C. for usually 10 minutes to 12 hours, preferably 30 minutes to 3 hours.

Specific examples of the fluoroalkylsilane compounds may include trifluoropropyl trimethoxysilane, tridecafluoroctyl trimethoxysilane, heptadecafluorodecyl trimethoxysilane, heptadecafluorodecylmethyl

5 dimethoxysilane, trifluoropropyl triethoxysilane, tridecafluoroctyl triethoxysilane, heptadecafluorodecyl triethoxysilane, heptadecafluorodecylmethyl diethoxysilane or the like. Among these fluoroalkylsilane compounds, in view of the desorption percentage and the adhering effect of

10 carbon black, trifluoropropyl trimethoxysilane, tridecafluoroctyl trimethoxysilane and heptadecafluorodecyl trimethoxysilane are preferred, and trifluoropropyl trimethoxysilane and tridecafluoroctyl trimethoxysilane are more preferred.

15 The amount of the coating layer composed of the organosilicon compounds is usually 0.02 to 5.0% by weight, preferably 0.03 to 4.0% by weight, more preferably 0.05 to 3.0% by weight (calculated as Si) based on the weight of the magnetic iron oxide particles coated with the organosilicon compounds.

When amount of the coating layer composed of the organosilicon compounds is less than 0.02% by weight, it becomes difficult to adhere the carbon black on the surfaces of the magnetic iron oxide particles in such an amount

25 enough to improve the fluidity and blackness of the obtained black magnetic composite particles.

On the other hand, when the coating amount of the organosilicon compounds is more than 5.0% by weight, a sufficient amount of the carbon black coat can be formed on the surfaces of the coating layer. However, the use of such unnecessarily large amount of the organosilicon compounds is meaningless because the effect of enhancing the fluidity or blackness of the obtained black magnetic composite particles is already saturated.

35 As the carbon black fine particles used in the present invention, there may be exemplified commercially available carbon blacks such as furnace black, channel black or the like. Specific examples of the commercially available carbon blacks usable in the present invention, may include

40 #3050, #3150, #3250, #3750, #3950, MA-100, MA7, #1000, #2400B, #30, MA8, MA11, #50, #52, #45, #2200B, MA600, etc. (tradename, produced by MITSUBISHI CHEMICAL CORP.), SEAST 9H, SEAST 7H, SEAST 6, SEAST 3H, SEAST 300, SEAST FM, etc. (tradename, produced by

45 TOKAI CARBON CO., LTD.), Raven 1250, Raven 860, Raven 1000, Raven 1190 ULTRA, etc. (tradename, produced by COLOMBIAN CHEMICALS COMPANY), Ketchen black EC, Ketchen black EC600JD, etc. (tradename, produced by KETCHEN INTERNATIONAL CO., LTD.), BLACK PEARLS-L, BLACK PEARLS 1000, BLACK PEARLS 4630, VULCAN XC72, REGAL 660, REGAL 400, etc. (tradename, produced by CABOTT SPECIALTY CHEMICALS INK CO., LTD.), or the like. In view of the compatibility with the organosilicon compounds, MA-100, MA7, #1000, #2400B and #30 are preferred.

50 The lower limit of the average particle size of the carbon black fine particles used is usually 0.002  $\mu m$ , preferably 0.005  $\mu m$ , and upper limit thereof is usually 0.05  $\mu m$ .

55 preferably 0.035  $\mu m$ . When the average particle size of the carbon black fine particles used is less than 0.002  $\mu m$ , the carbon black fine particles used are too fine to be well handled.

On the other hand, when the average particle size thereof is more than 0.05  $\mu m$ , since the particle size of the carbon black fine particles used is much larger, it is necessary to apply a larger mechanical shear force for forming the

uniform carbon black coat on the coating layer composed of the organosilicon compounds, thereby rendering the coating process industrially disadvantageous.

The amount of the carbon black coat formed is 1 to 25 parts by weight based on 100 parts by weight of the magnetic iron oxide particles as core particles.

When the amount of the carbon black coat formed is less than 1 part by weight, the amount of the carbon black is insufficient, so that it becomes difficult to obtain black magnetic composite particles having a sufficient fluidity and blackness.

On the other hand, when the amount of the carbon black coat formed is more than 25 parts by weight, the obtained black magnetic composite particles can show a sufficient fluidity and blackness. However, since the amount of the carbon black is considerably large, the carbon black tend to be desorbed from the coating layer composed of the organosilicon compound. As a result, the obtained black magnetic composite particles tend to be deteriorated in dispersibility in a binder resin upon the production of magnetic toner.

The thickness of carbon black coat formed is preferably not more than 0.04  $\mu\text{m}$ , more preferably not more than 0.03  $\mu\text{m}$ , still more preferably not more than 0.02  $\mu\text{m}$ . The lower limit thereof is more preferably 0.0001  $\mu\text{m}$ .

In the black magnetic composite particles according to the present invention, at least a part of the surface of the magnetic iron oxide particle as core particle may be preliminarily coated with at least one compound selected from the group consisting of hydroxides of aluminum, oxides of aluminum, hydroxides of silicon and oxides of silicon (hereinafter referred to as "hydroxides and/or oxides of aluminum and/or silicon coat"), if necessary. In this case, the obtained black magnetic composite particles can show a higher dispersibility in a binder resin as compared to in the case where the magnetic iron oxide particles are uncoated with hydroxides and/or oxides of aluminum and/or silicon.

The amount of the hydroxides and/or oxides of aluminum and/or silicon coat is preferably 0.01 to 50% by weight (calculated as Al,  $\text{SiO}_2$  or a sum of Al and  $\text{SiO}_2$ ) based on the weight of the magnetic iron oxide particles as core particles.

When the amount of the hydroxides and/or oxides of aluminum and/or silicon coat is less than 0.01% by weight, the effect of enhancing the dispersibility of the obtained black magnetic composite particles in a binder resin upon the production of magnetic toner cannot be obtained.

On the other hand, when the amount of the hydroxides and/or oxides of aluminum and/or silicon coat is more than 50% by weight, the obtained black magnetic composite particles can exhibit a good dispersibility in a binder resin upon the production of magnetic toner. However, such unnecessarily large amount of the hydroxides and/or oxides of aluminum and/or silicon coat is meaningless.

The particle size, geometrical standard deviation, BET specific surface area, fluidity, blackness L\* value and desorption percentage of carbon black of the black magnetic composite particles wherein the surface of the core particle is coated with the hydroxides and/or oxides of aluminum and/or silicon according to the present invention, are substantially the same as those of the black magnetic composite particles wherein the core particle is uncoated with the hydroxides and/or oxides of aluminum and/or silicon according to the present invention.

The black magnetic composite particles used for the black magnetic toner according to the present invention can be produced by the following method.

Among the isotropic magnetite particles which are magnetic iron oxide particles, (1) octahedral magnetite particles can be produced by passing an oxygen-containing gas through a suspension containing ferrous hydroxide colloid having a pH value of not less than 10, which is obtained by reacting an aqueous ferrous salt solution with an aqueous alkali solution having a concentration of not less than one equivalent based on  $\text{Fe}^{2+}$  in the aqueous ferrous salt solution, thereby precipitating magnetite particles, and then 5 subjecting the obtained magnetite particles to filtering, washing with water and drying (Japanese Patent Publication (KOKOKU) No. 44-668(1969); (2) hexahedral magnetite particles can be produced by passing an oxygen-containing gas through a suspension containing ferrous hydroxide colloid having a pH value of 6.0 to 7.5, which is obtained by 10 reacting an aqueous ferrous salt solution with an aqueous alkali solution having a concentration of not more than one equivalent based on  $\text{Fe}^{2+}$  in the aqueous ferrous salt solution to produce magnetite core particles, further passing an oxygen-containing gas through the obtained aqueous ferrous salt reaction solution containing the magnetite core particles and the ferrous hydroxide colloid, at a pH value of 8.0 to 9.5, 15 to precipitate magnetite particles, and then subjecting the precipitated magnetite particles to filtering, washing with water and drying (Japanese Patent Application Laid-Open (KOKAI) No. 3 -201509(1991); (3) spherical magnetite particles can be produced by passing an oxygen-containing gas through a suspension containing ferrous hydroxide colloid having a pH value of 6.0 to 7.5, which is obtained by 20 reacting an aqueous ferrous salt solution with an aqueous alkali solution having a concentration of not more than one equivalent based on  $\text{Fe}^{2+}$  in the aqueous ferrous salt solution to produce magnetite core particles, adding alkali hydroxide in an amount of not less than equivalent based on the 25 remaining  $\text{Fe}^{2+}$  to adjust the pH value of the suspension to not less than 10, heat-oxidizing the resultant suspension to precipitate magnetite particles, and then subjecting the precipitated magnetite particles to filtering, washing with water and drying (Japanese Patent Publication (KOKOKU) No. 62-51208(1987).

The isotropic maghemite particles can be obtained by heating the above-mentioned isotropic magnetite particles in air at 300 to 600°C.

The anisotropic magnetite particles can be produced by 45 passing an oxygen-containing gas through a suspension containing either ferrous hydroxide colloid, iron carbonate, or an iron-containing precipitate obtained by reacting an aqueous ferrous salt solution with alkali hydroxide and/or alkali carbonate, while appropriately controlling the pH 50 value and temperature of the suspension, to produce acicular, spindle-shaped or rice ball-shaped goethite particles, subjecting the obtained goethite particles to filtering, washing with water and drying, and then reducing the goethite particles in a heat-reducing gas at 300 to 800°C.

The anisotropic maghemite particles can be produced by heat-oxidizing the above-mentioned anisotropic magnetite particles in an oxygen-containing gas at 300 to 600°C.

The coating of the magnetic iron oxide particles with the 60 alkoxy silane compounds, the polysiloxanes, the modified polysiloxanes, the terminal-modified polysiloxanes or the fluoroalkylsilane compounds, may be conducted (i) by mechanically mixing and stirring the magnetic iron oxide particles together with the alkoxy silane compounds, the polysiloxanes, the modified polysiloxanes, the terminal-modified polysiloxanes or the fluoroalkylsilane compounds; or (ii) by mechanically mixing and stirring both the com- 65

ponents together while spraying the alkoxy silane compounds, the polysiloxanes, the modified polysiloxanes, the terminal-modified polysiloxanes or the fluoroalkylsilane compounds onto the magnetic iron oxide particles. In these cases, substantially whole amount of the alkoxy silane compounds, the polysiloxanes, the modified polysiloxanes, the terminal-modified polysiloxanes or the fluoroalkylsilane compounds added can be applied onto the surfaces of the magnetic iron oxide particles.

In order to uniformly coat the surfaces of the magnetic iron oxide particles with the alkoxy silane compounds, the polysiloxanes, the modified polysiloxanes, the terminal-modified polysiloxanes or the fluoroalkylsilane compounds, it is preferred that the magnetic iron oxide particles are preliminarily disaggregated by using a pulverizer.

As apparatus (a) for mixing and stirring the core particles with the alkoxy silane compounds, the polysiloxanes, the modified polysiloxanes, the terminal-modified polysiloxanes or the fluoroalkylsilane compounds to form the coating layer thereof, and (b) for mixing and stirring carbon black fine particles with the particles whose surfaces are coated with the alkoxy silane compounds, the polysiloxanes, the modified polysiloxanes, the terminal-modified polysiloxanes or the fluoroalkylsilane compounds to form the carbon black coat, there may be preferably used those apparatus capable of applying a shear force to the particles, more preferably those apparatuses capable of conducting the application of shear force, spatulate-force and compressed-force at the same time. In addition, by conducting the above mixing or stirring treatment (a) of the core particles together with the alkoxy silane compounds, the polysiloxanes, the modified polysiloxanes, the terminal-modified polysiloxanes or the fluoroalkylsilane compounds, at least a part of the alkoxy silane compounds and the fluoroalkylsilane compounds coated on the core particles may be changed to the organosilane compounds and fluoroalkyl organosilane compounds, respectively.

As such apparatuses, there may be exemplified wheel-type kneaders, ball-type kneaders, blade-type kneaders, roll-type kneaders or the like. Among them, wheel-type kneaders are preferred.

Specific examples of the wheel-type kneaders may include an edge runner (equal to a mix muller, a Simpson mill or a sand mill), a multi-mull, a Stotz mill, a wet pan mill, a Conner mill, a ring muller, or the like. Among them, an edge runner, a multi-mull, a Stotz mill, a wet pan mill and a ring muller are preferred, and an edge runner is more preferred. Specific examples of the ball-type kneaders may include a vibrating mill or the like. Specific examples of the blade-type kneaders may include a Henschel mixer, a planetary mixer, a Nawter mixer or the like. Specific examples of the roll-type kneaders may include an extruder or the like.

In order to coat the surfaces of the core particles with the alkoxy silane compounds, the polysiloxanes, the modified polysiloxanes, the terminal-modified polysiloxanes or the fluoroalkylsilane compounds as uniformly as possible, the conditions of the above mixing or stirring treatment may be appropriately controlled such that the linear load is usually 2 to 200 Kg/cm, preferably 10 to 150 kg/cm, more preferably 15 to 100 kg/cm; and the treating time is usually 5 to 120 minutes, preferably 10 to 90 minutes. It is preferred to appropriately adjust the stirring speed in the range of usually 2 to 2,000 rpm, preferably 5 to 1,000 rpm, more preferably 10 to 800 rpm.

The amount of the alkoxy silane compounds, the polysiloxanes, the modified polysiloxanes, the terminal-modified polysiloxanes or the fluoroalkylsilane compounds

added, is preferably 0.15 to 45 parts by weight based on 100 parts by weight of the magnetic iron oxide particles. When the amount of the alkoxy silane compounds, the polysiloxanes, the modified polysiloxanes, the terminal-modified polysiloxanes or the fluoroalkylsilane compounds added is less than 0.15 part by weight, it may become difficult to form the carbon black coat in such an amount enough to improve the blackness and flowability of the obtained black magnetic composite particles.

On the other hand, when the amount of the alkoxy silane compounds, the polysiloxanes, the modified polysiloxanes, the terminal-modified polysiloxanes or the fluoroalkylsilane compounds added is more than 45 parts by weight, a sufficient amount of the carbon black coat can be formed on the surface of the coating, but it is meaningless because the blackness and flowability of the composite particles cannot be further improved by using such an excess amount of the alkoxy silane compounds, the polysiloxanes, the modified polysiloxanes, the terminal-modified polysiloxanes or the fluoroalkylsilane compounds added.

Next, the carbon black fine particles are added to the magnetic iron oxide particles coated with the alkoxy silane compounds, the polysiloxanes, the modified polysiloxanes, the terminal-modified polysiloxanes or the fluoroalkylsilane compounds, and the resultant mixture is mixed and stirred to form the carbon black coat on the surfaces of the coating composed of the alkoxy silane compounds, the polysiloxanes, the modified polysiloxanes, the terminal-modified polysiloxanes or the fluoroalkylsilane compounds added. In addition, by conducting the above mixing or stirring treatment (b) of the carbon black fine particles together with the magnetic iron oxide particles coated with the alkoxy silane compounds, the polysiloxanes, the modified polysiloxanes, the terminal-modified polysiloxanes or the fluoroalkylsilane compounds, at least a part of the alkoxy silane compounds and the fluoroalkylsilane compounds coated on the magnetic iron oxide particles may be changed to the organosilane compounds and fluoroalkyl organosilane compounds, respectively.

In the case where the alkoxy silane compounds and the fluoroalkylsilane compounds are used as the coating compound, after the carbon black coat is formed on the surface of the coating layer, the resultant composite particles may be dried or heat-treated, for example, at a temperature of usually 40 to 200° C., preferably 60 to 150° C. for usually 10 minutes to 12 hours, preferably 30 minutes to 3 hours, thereby forming a coating layer composed of the organosilane compounds (1) and the fluoroalkyl organosilane compounds (3), respectively.

It is preferred that the carbon black fine particles are added little by little and slowly, especially about 5 to 60 minutes.

In order to form carbon black onto the coating layer composed of the alkoxy silane compounds, the polysiloxanes, the modified polysiloxanes, the terminal-modified polysiloxanes or the fluoroalkylsilane compounds as uniformly as possible, the conditions of the above mixing or stirring treatment can be appropriately controlled such that the linear load is usually 2 to 200 Kg/cm, preferably 10 to 150 Kg/cm more preferably 15 to 100 Kg/cm; and the treating time is usually 5 to 120 minutes, preferably 10 to 90 minutes. It is preferred to appropriately adjust the stirring speed in the range of usually 2 to 2,000 rpm, preferably 5 to 1,000 rpm, more preferably 10 to 800 rpm.

The amount of the carbon black fine particles added, is preferably 1 to 25 parts by weight based on 100 parts by weight of the magnetic iron oxide particles. When the

amount of the carbon black fine particles added is less than 1 part by weight, it may become difficult to form the carbon black coat in such an amount enough to improve the blackness and flowability of the obtained composite particles. On the other hand, when the amount of the carbon black fine particles added is more than 25 parts by weight, a sufficient blackness and flowability of the resultant composite particles can be obtained, but the carbon black tend to be desorbed from the surface of the coating layer because of too large amount of the carbon black adhered, resulting in deteriorated dispersibility in the binder resin upon the production of the magnetic toner.

At least a part of the surface of the magnetic iron oxide particles may be coated with at least one compound selected from the group consisting of hydroxides of aluminum, oxides of aluminum, hydroxides of silicon and oxides of silicon, if required, in advance of mixing and stirring with the alkoxysilane compounds, the polysiloxanes, the modified polysiloxanes, the terminal-modified polysiloxanes or the fluoroalkylsilane compounds.

The coat of the hydroxides and/or oxides of aluminum and/or silicon may be conducted by adding an aluminum compound, a silicon compound or both the compounds to a water suspension in which the magnetic iron oxide particles are dispersed, followed by mixing and stirring, and further adjusting the pH value of the suspension, if required, thereby coating the surfaces of the magnetic iron oxide particles with at least one compound selected from the group consisting of hydroxides of aluminum, oxides of aluminum, hydroxides of silicon and oxides of silicon. The thus obtained particles coated with the hydroxides and/or oxides of aluminum and/or silicon are then filtered out, washed with water, dried and pulverized. Further, the particles coated with the hydroxides and/or oxides of aluminum and/or silicon may be subjected to post-treatments such as deaeration treatment and compaction treatment, if required.

As the aluminum compounds, there may be exemplified aluminum salts such as aluminum acetate, aluminum sulfate, aluminum chloride or aluminum nitrate, alkali aluminates such as sodium aluminate, alumina sols or the like.

The amount of the aluminum compound added is 0.01 to 50% by weight (calculated as Al) based on the weight of the magnetic iron oxide particles. When the amount of the aluminum compound added is less than 0.01% by weight, it may be difficult to sufficiently coat the surfaces of the magnetic iron oxide particles with hydroxides and/or oxides of aluminum, thereby failing to achieve the improvement of the dispersibility in the binder resin upon the production of the magnetic toner. On the other hand, when the amount of the aluminum compound added is more than 50% by weight, the coating effect is saturated and, therefore, it is meaningless to add such an excess amount of the aluminum compound.

As the silicon compounds, there may be exemplified water glass #3, sodium orthosilicate, sodium metasilicate, colloidal silica or the like.

The amount of the silicon compound added is 0.01 to 50% by weight (calculated as SiO<sub>2</sub>) based on the weight of the magnetic iron oxide particles. When the amount of the silicon compound added is less than 0.01% by weight, it may be difficult to sufficiently coat the surfaces of the magnetic iron oxide particles with hydroxides and/or oxides of silicon, thereby failing to achieve the improvement of the dispersibility in the binder resin upon the production of the magnetic toner. On the other hand, when the amount of the silicon compound added is more than 50% by weight, the coating effect is saturated and, therefore, it is meaningless to add such an excess amount of the silicon compound.

In the case where both the aluminum and silicon compounds are used in combination for the coating, the total amount of the aluminum and silicon compounds added is preferably 0.01 to 50% by weight (calculated as a sum of Al and SiO<sub>2</sub>) based on the weight of the magnetic iron oxide particles.

Next, the black magnetic toner according to the present invention is described.

The black magnetic toner according to the present invention 10 comprises the black magnetic composite particles, and a binder resin. The black magnetic toner may further contain a mold release agent, a colorant, a charge-controlling agent and other additives, if necessary.

The black magnetic toner according to the present invention 15 has an average particle size of usually 3 to 15  $\mu\text{m}$ , preferably 5 to 12  $\mu\text{m}$ .

The amount of the binder resin used in the black magnetic toner is usually 50 to 900 parts by weight, preferably 50 to 400 parts by weight based on 100 parts by weight of the 20 black magnetic composite particles.

As the binder resins, there may be used vinyl-based polymers, i.e., homopolymers or copolymers of vinyl-based monomers such as styrene, alkyl acrylates and alkyl methacrylates. As the styrene monomers, there may be exemplified styrene and substituted styrenes. As the alkyl acrylate monomers, there may be exemplified acrylic acid, methyl acrylate, ethyl acrylate, butyl acrylate or the like.

It is preferred that the above copolymers contain styrene-based components in an amount of usually 50 to 95% by weight.

In the binder resin used in the present invention, the above-mentioned vinyl-based polymers may be used in combination with polyester-based resins, epoxy-based resins, polyurethane-based resins or the like, if necessary.

As to the fluidity of the black magnetic toner according to the present invention, the fluidity index is usually 70 to 100, preferably 71 to 100, more preferably 72 to 100. When the fluidity index is less than 70, the black magnetic toner may not show a sufficient fluidity.

The blackness of the black magnetic toner according to the present invention is usually not more than 20, preferably not more than 19.8, more preferably not more than 19.5 when represented by L\* value. When the blackness thereof is more than 20, the lightness of the black magnetic toner may be increased, resulting in insufficient blackness. The lower limit of the blackness of the black magnetic toner is usually about 15 when represented by L\* value.

The volume resistivity of the black magnetic toner according to the present invention, is usually not less than 1.0 $\times 10^{13}$   $\Omega\cdot\text{cm}$ , preferably not less than 3.0 $\times 10^{13}$   $\Omega\cdot\text{cm}$ , more preferably not less than 5.0 $\times 10^{13}$   $\Omega\cdot\text{cm}$ . When the volume resistivity is less than 1.0 $\times 10^{13}$   $\Omega\cdot\text{cm}$ , the charge amount of the black magnetic toner tends to vary depending upon environmental conditions in which the toner is used, resulting in unstable properties of the black magnetic toner. The upper limit of the volume resistivity is 1.0 $\times 10^{15}$   $\Omega\cdot\text{cm}$ .

As to the magnetic properties of the black magnetic toner according to the present invention, the coercive force thereof is usually 10 to 350 Oe, preferably 20 to 330 Oe; the 60 saturation magnetization value in a magnetic field of 10 kOe is usually 10 to 85 emu/g, preferably 20 to 80 emu/g; the residual magnetization in a magnetic field of 10 kOe is usually 1 to 20 emu/g, preferably 2 to 15 emu/g; the saturation magnetization in a magnetic field of 1 kOe is usually 7.5 to 65 emu/g, preferably 10 to 60 emu/g; and the residual magnetization in a magnetic field of 1 kOe is usually 0.5 to 15 emu/g, preferably 1.0 to 13 emu/g.

The black magnetic toner according to the present invention may be produced by a known method of mixing and kneading a predetermined amount of a binder resin and a predetermined amount of the black magnetic composite particles together, and then pulverizing the mixed and kneaded material into particles. More specifically, the black magnetic composite particles and the binder resin are intimately mixed together with, if necessary, a mold release agent, a colorant, a charge-controlling agent or other additives by using a mixer. The obtained mixture is then melted and kneaded by a heating kneader so as to render the respective components compatible with each other, thereby dispersing the black magnetic composite particles therein. Successively, the molten mixture is cooled and solidified to obtain a resin mixture. The obtained resin mixture is then pulverized and classified, thereby producing a magnetic toner having an aimed particle size.

As the mixers, there may be used a Henschel mixer, a ball mill or the like. As the heating kneaders, there may be used a roll mill, a kneader, a twin-screw extruder or the like. The pulverization of the resin mixture may be conducted by using pulverizers such as a cutter mill, a jet mill or the like. The classification of the pulverized particles may be conducted by known methods such as air classification, etc., as described in Japanese Patent No. 2683142 or the like.

As the other method of producing the black magnetic toner, there may be exemplified a suspension polymerization method or an emulsion polymerization method. In the suspension polymerization method, polymerizable monomers and the black magnetic composite particles are intimately mixed together with, if necessary, a colorant, a polymerization initiator, a cross-linking agent, a charge-controlling agent or the other additives and then the obtained mixture is dissolved and dispersed together so as to obtain a monomer composition. The obtained monomer composition is added to a water phase containing a suspension stabilizer while stirring, thereby granulating and polymerizing the composition to form magnetic toner particles having an aimed particle size.

In the emulsion polymerization method, the monomers and the black magnetic composite particles are dispersed in water together with, if necessary, a colorant, a polymerization initiator or the like and then the obtained dispersion is polymerized while adding an emulsifier thereto, thereby producing magnetic toner particles having an aimed particle size.

A point of the present invention exists in that the black magnetic composite particles comprising as core particles the magnetic iron oxide particles which have an average particle size of 0.055 to 0.95  $\mu\text{m}$  and may be coated with at least one compound selected from the group consisting of hydroxides of aluminum, oxides of aluminum, hydroxides of silicon and oxides of silicon; the organosilicon compounds coated on the surface of the magnetic iron oxide particle; the carbon black coat formed on the surface of the coating layer composed of the organosilicon compounds in an amount of 1 to 25 parts by weight based on 100 parts by weight of the magnetic iron oxide particles, can show not only excellent fluidity and blackness, but also an excellent dispersibility in a binder resin upon the production of magnetic toner due to less amount of carbon black desorbed or fallen-off from the surfaces of the particles.

The reason why the amount of the carbon black desorbed or fallen-off from the surfaces of the black magnetic composite particles according to the present invention, is small, is considered as follows. That is, the organosilicon compounds and the surfaces of the magnetic iron oxide particles

are strongly bonded to each other, so that the carbon black bonded to the surfaces of the magnetic iron oxide particles through the organosilicon compounds can be prevented from being desorbed from the magnetic iron oxide particles.

In particular, in the case of the alkoxy silane compounds (1) and the fluoroalkyl silane compounds (3), metalloxane bonds ( $\equiv\text{Si}—\text{O}—\text{M}$  wherein M represents a metal atom contained in the black iron oxide particles, such as Si, Al, Fe or the like) are formed between the surfaces of the magnetic iron oxide particles and alkoxy groups contained in the organosilicon compounds onto which the carbon black coat is formed, thereby forming a stronger bond between the organosilicon compounds on which the carbon black coat is formed, and the surfaces of the magnetic iron oxide particles.

The reason why the black magnetic composite particles according to the present invention can show an excellent dispersibility in a binder resin upon the production of magnetic toner, is considered such that since only a small amount of the carbon black is desorbed or fallen-off from the surfaces of the black magnetic composite particles, the black magnetic composite particles is free from deterioration in dispersibility due to the desorbed or fallen-off carbon black, and further since the carbon black coat is formed on the surfaces of the black magnetic composite particles and, therefore, irregularities are formed on the surfaces of the black magnetic composite particles, the contact between the particles can be suppressed.

The reason why the black magnetic composite particles according to the present invention can show an excellent fluidity, is considered as follows. That is, the carbon black fine particles which are ordinarily agglomerated together due to fineness thereof, are allowed to be uniformly and densely formed on the surfaces of the magnetic iron oxide particles and, therefore, can be dispersed nearly in the form of primary particles, so that many fine irregularities are formed on the surfaces of the magnetic iron oxide particles.

The reason why the black magnetic composite particles according to the present invention can show an excellent blackness, is considered such that since the carbon black coat are uniformly and densely formed on the surfaces of the magnetic iron oxide particles, the color tone of the core particles is hidden behind the carbon black, so that an inherent color tone of carbon black can be exhibited.

Therefore, the black magnetic toner produced by using the above black magnetic composite particles, can show excellent fluidity and blackness.

The reason why the black magnetic toner according to the present invention can show an excellent fluidity, is considered as follows. That is, the black magnetic composite particles on which a large amount of the carbon black is uniformly formed, are blended in the black magnetic toner, so that many fine irregularities are formed on the surface of the black magnetic toner.

The reason why the black magnetic toner according to the present invention can show an excellent blackness, is considered such that the black magnetic composite particles having an excellent blackness is blended in the black magnetic toner.

As described above, since the black magnetic composite particles according to the present invention, are excellent not only in fluidity and blackness, but also in dispersibility in a binder resin due to less amount of the carbon black desorbed or fallen-off from the surfaces thereof, the black magnetic composite particles according to the present invention, are suitable as black magnetic particles for black magnetic toner capable of attaining a high image quality and a high copying speed.

In addition, since the black magnetic composite particles according to the present invention, are excellent in dispersibility in a binder resin, the particles can show excellent handling property and workability and, therefore, are preferable from an industrial viewpoint.

Further, the black magnetic toner produced from the above black magnetic composite particles which are excellent in fluidity and blackness, can also show excellent fluidity and blackness. Accordingly, the black magnetic toner is suitable as black magnetic toner capable of attaining a high image quality and a high copying speed.

Furthermore, in the black magnetic toner according to the present invention, since the black magnetic composite particles contained therein are excellent in dispersibility, it is possible to expose the black magnetic composite particles to the surface of the black magnetic toner independently and separately. As a result, the black magnetic toner can be free from being deteriorated in electric resistance due to the existence of the carbon black coat. Accordingly, the black magnetic toner according to the present invention is suitable as a high-resistance or insulated magnetic toner.

#### EXAMPLES

The present invention is described in more detail by Examples and Comparative Examples, but the Examples are only illustrative and, therefore, not intended to limit the scope of the present invention.

Various properties were measured by the following methods.

(1) The average particle size, the average major axial diameter and average minor axial diameter of magnetite particles, maghemite particles, black magnetic composite particles and carbon black fine particles were respectively expressed by the average of values (measured in a predetermined direction) of about 350 particles which were sampled from a micrograph obtained by magnifying an original electron micrograph ( $\times 20,000$ ) by four times in each of the longitudinal and transverse directions.

(2) The aspect ratio of the particles was expressed by the ratio of average major axial diameter to average minor axial diameter thereof.

(3) The geometrical standard deviation of particle sizes was expressed by values obtained by the following method. That is, the particle sizes (major axial diameters) were measured from the above magnified electron micrograph. The actual particle sizes (major axial diameters) and the number of the particles were calculated from the measured values. On a logarithmic normal probability paper, the particle sizes (major axial diameters) were plotted at regular intervals on the abscissa-axis and the accumulative number (under integration sieve) of particles belonging to each interval of the particle sizes (major axial diameters) were plotted by percentage on the ordinate-axis by a statistical technique.

The particle sizes (major axial diameters) corresponding to the number of particles of 50% and 84.13%, respectively, were read from the graph, and the geometrical standard deviation was calculated from the following formula:

$$\text{Geometrical standard deviation} = \frac{\{\text{particle size (major axial diameters) corresponding to 84.13\% under integration sieve}\} - \{\text{particle size (major axial diameters) (geometrical average diameter) corresponding to 50\% under integration sieve}\}}{\{\text{particle size (major axial diameters) (geometrical average diameter) corresponding to 50\% under integration sieve}\}}$$

The closer to 1 the geometrical standard deviation value, the more excellent the particle size distribution.

(4) The specific surface area was expressed by the value measured by a BET method.

(5) The amounts of Al and Si which were present within black magnetic composite particles or on surfaces thereof, and the amount of Si contained in the organosilicon compounds, were measured by a fluorescent X-ray spectroscopy device 3063 (manufactured by Rigaku Denki Kogyo Co., Ltd.) according to JIS K0119 "General rule of fluorescent X-ray analysis".

(6) The amount of carbon black coat formed on the surface of the black magnetic composite particles was measured by "Horiba Metal, Carbon and Sulfur Analyzer EMIA-2200 Model" (manufactured by Horiba Seisakusho Co., Ltd.).

(7) The thickness of carbon black coat formed on the surfaces of the black magnetic composite particles is expressed by the value which was obtained by first measuring an average thickness of carbon black coat formed onto the surfaces of the particles on a photograph ( $\times 5,000,000$ ) obtained by magnifying (ten times) a micrograph ( $\times 500,000$ ) produced at an accelerating voltage of 200 kV using a transmission-type electron microscope (JEM-2010, manufactured by Japan Electron Co., Ltd.), and then calculating an actual thickness of carbon black coat formed from the measured average thickness.

(8) The fluidity of magnetic iron oxide particles, black magnetic composite particles and magnetic toner was expressed by a fluidity index which was a sum of indices obtained by converting on the basis of the same reference measured values of an angle of repose, a degree of compaction (%), an angle of spatula and a degree of agglomeration as particle characteristics which were measured by a powder tester (tradename, produced by Hosokawa Micron Co., Ltd.). The closer to 100 the fluidity index, the more excellent the fluidity of the particles.

(9) The blackness of magnetic iron oxide particles, black magnetic composite particles and magnetic toner was measured by the following method. That is, 0.5 g of sample particles and 1.5 ml of castor oil were intimately kneaded together by a Hoover's muller to form a paste. 4.5 g of clear lacquer was added to the obtained paste and was intimately kneaded to form a paint. The obtained paint was applied on a cast-coated paper by using a 6-mil (150  $\mu\text{m}$ ) applicator to produce a coating film piece (having a film thickness of about 30  $\mu\text{m}$ ). The thus obtained coating film piece was measured according to JIS Z 8729 by a multi-light source spectrographic calorimeter MSC-IS-2D (manufactured by Suga Testing Machines Manufacturing Co., Ltd.) to determine an  $L^*$  value of calorimetric indices thereof. The blackness was expressed by the  $L^*$  value measured.

Here, the  $L^*$  value represents a lightness, and the smaller the  $L^*$  value, the more excellent the blackness.

(10) The desorption percentage of carbon black desorbed from the black magnetic composite particles was measured by the following method. The closer to zero the desorption percentage, the smaller the amount of carbon black desorbed from the surfaces of black magnetic composite particles.

That is, 3 g of the black magnetic composite particles and 40 ml of ethanol were placed in a 50-ml precipitation pipe and then was subjected to ultrasonic dispersion for 20 minutes. Thereafter, the obtained dispersion was allowed to stand for 120 minutes, and the carbon black desorbed were separated from the black magnetic composite particles on the basis of the difference in specific gravity between both the particles. Next, the black magnetic composite particles from which the desorbed carbon black was separated, were mixed again with 40 ml of ethanol, and the obtained mixture was further subjected to ultrasonic dispersion for 20 minutes. Thereafter, the obtained dispersion was allowed to

stand for 120 minutes, thereby separating the black magnetic composite particles and the desorbed carbon black desorbed from each other. The thus obtained black magnetic composite particles were dried at 100° C. for one hour, and then the carbon content thereof was measured by the "Horiba Metal, Carbon and Sulfur Analyzer EMIA-2200 Model" (manufactured by Horiba Seisakusho Co., Ltd.). The desorption percentage of the carbon black was calculated according to the following formula:

$$\text{Desorption percentage of carbon black (\%)} = \{(W_a - W_e)/W_a\} \times 100$$

wherein  $W_a$  represents an amount of carbon black initially formed on the black magnetic composite particles; and  $W_e$  represents an amount of carbon black still adhered on the black magnetic composite particles after desorption test.

(11) The dispersibility in a binder resin of the black magnetic composite particles was evaluated by counting the number of undispersed agglomerated particles on a micrograph ( $\times 200$  times) obtained by photographing a sectional area of the obtained black magnetic toner particle using an optical microscope (BH-2, manufactured by Olympus Kogaku Kogyo Co., Ltd.), and classifying the results into the following five ranks. The 5th rank represents the most excellent dispersing condition.

Rank 1: not less than 50 undispersed agglomerated particles per  $0.25 \text{ mm}^2$  were recognized;

Rank 2: 10 to 49 undispersed agglomerated particles per  $0.25 \text{ mm}^2$  were recognized;

Rank 3: 5 to 9 undispersed agglomerated particles per  $0.25 \text{ mm}^2$  were recognized;

Rank 4: 1 to 4 undispersed agglomerated particles per  $0.25 \text{ mm}^2$  were recognized;

Rank 5: No undispersed agglomerated particles were recognized.

(12) The average particle size of the black magnetic toner was measured by a laser diffraction-type particle size distribution-measuring apparatus (Model HELOSLA/KA, manufactured by Sympatec Corp.).

(13) The volume resistivity of the magnetic iron oxide particles, the black magnetic composite particles and the black magnetic toner was measured by the following method.

That is, first, 0.5 g of a sample particles or toner to be measured was weighted, and press-molded at 140 Kg/cm<sup>2</sup> using a KBr tablet machine (manufactured by Simazu Seisakusho Co., Ltd.), thereby forming a cylindrical test piece.

Next, the thus obtained cylindrical test piece was exposed to an atmosphere maintained at a temperature of 25° C. and a relative humidity of 60% for 12 hours. Thereafter, the cylindrical test piece was set between stainless steel electrodes, and a voltage of 15V was applied between the electrodes using a Wheatstone bridge (TYPE2768, manufactured by Yokogawa-Hokushin Denki Co., Ltd.) to measure a resistance value  $R$  (Ω).

The cylindrical test piece was measured with respect to an upper surface area  $A$  (cm<sup>2</sup>) and a thickness  $t_0$  (cm) thereof. The measured values were inserted into the following formula, thereby obtaining a volume resistivity  $X$  (Ω·cm).

$$X(\Omega \cdot \text{cm}) = R \times (A/t_0)$$

(14) The magnetic properties of the magnetic iron oxide particles and the black magnetic composite particles were measured using a vibration sample magnetometer "VSM-3S-15" (manufactured by Toei Kogyo Co., Ltd.) by applying an external magnetic field of 10 kOe thereto. Whereas, the

magnetic properties of the black magnetic toner were measured by applying external magnetic fields of 1 kOe and 10 kOe thereto.

#### Example 1

##### 5 <Production of Black Magnetic Composite Particles>

20 kg of spherical magnetite particles shown in the electron micrograph ( $\times 20,000$ ) of FIG. 1 (average particle size: 0.23 μm; geometrical standard deviation value: 1.42; BET specific surface area value: 9.2 m<sup>2</sup>/g; blackness (L\* value): 20.6; fluidity index: 35; coercive force value: 61 Oe; saturation magnetization value in a magnetic field of 10 kOe: 84.9 emu/g; residual magnetization value in a magnetic field of 10 kOe: 7.8 emu/g), were deagglomerated in 150 liters of pure water using a stirrer, and further passed through

15 a "TK pipeline homomixer" (tradename, manufactured by Tokushu Kika Kogyo Co., Ltd.) three times, thereby obtaining a slurry containing the spherical magnetite particles.

25 Successively, the obtained slurry containing the spherical magnetite particles was passed through a transverse-type sand grinder (tradename "MIGHTY MILL MHG-1.5L", manufactured by Inoue Seisakusho Co., Ltd.) five times at an axis-rotating speed of 2,000 rpm, thereby obtaining a slurry in which the spherical magnetite particles were dispersed.

20 The particles in the obtained slurry which remained on a sieve of 325 meshes (mesh size: 44 μm) was 0%. The slurry was filtered and washed with water, thereby obtaining a filter cake containing the spherical magnetite particles. After the obtained filter cake containing the spherical magnetite particles was dried at 120° C., 11.0 kg of the dried particles were then charged into an edge runner "MPUV-2 Model" (tradename, manufactured by Matsumoto Chuzo Tekkosho Co., Ltd.), and mixed and stirred at 30 Kg/cm and a stirring speed of 22 rpm for 30 minutes, thereby lightly deagglomerating the particles.

25 35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9

composite particles was 7.5%. As to the magnetic properties, the coercive force value of the black magnetic composite particles was 61 Oe; the saturation magnetization value in a magnetic field of 10 kOe was 77.3 emu/g; and the residual magnetization value in a magnetic field of 10 kOe was 7.1 emu/g. The coating amount of an organosilane compound produced from methyl triethoxysilane was 0.31% by weight calculated as Si. The amount of the carbon black coat formed on the coating layer composed of the organosilane compound produced from methyl triethoxysilane is 8.19% by weight (calculated as C) based on the weight of the black magnetic composite particles (corresponding to 9 parts by weight based on 100 parts by weight of the spherical magnetite particles). The thickness of the carbon black coat formed was 0.0024  $\mu\text{m}$ . Since no independent carbon black was observed on the electron micrograph of FIG. 3, it was determined that a whole amount of the carbon black used contributed to the formation of the carbon black coat on the coating layer composed of the organosilane compound produced from methyl triethoxysilane.

## Example 2

## &lt;Production of Black Magnetic Toner Containing Black Magnetic Composite Particles&gt;

400 g of the black magnetic composite particles obtained in Example 1, 540 g of styrene-butyl acrylate-methyl methacrylate copolymer resin (molecular weight=130,000, styrene/butyl acrylate/methyl methacrylate =82.0/16.5/1.5), 60 g of polypropylene wax (molecular weight: 3,000) and 15 g of a charge-controlling agent were charged into a Henschel mixer, and mixed and stirred therein at 60° C. for 15 minutes. The obtained mixed particles were melt-kneaded at 140° C. using a continuous-type twin-screw kneader (T-1), and the obtained kneaded material was cooled, coarsely pulverized and finely pulverized in air. The obtained particles were subjected to classification, thereby producing a black magnetic toner.

The obtained black magnetic toner had an average particle size of 9.7  $\mu\text{m}$ , a dispersibility of 5th rank, a fluidity index of 73, a blackness (L\* value) of 18.3, a volume resistivity of  $1.0 \times 10^{14} \Omega\cdot\text{cm}$ , a coercive force value of 60 Oe, a saturation magnetization value (in a magnetic field of 10 kOe) of 32.6 emu/g, a residual magnetization value (in a magnetic field of 10 kOe) of 4.3 emu/g, a saturation magnetization value (in a magnetic field of 1 kOe) of 25.9 emu/g, and a residual magnetization value (in a magnetic field of 1 kOe) of 3.5 emu/g.

## Example 3

## &lt;Production of Black Magnetic Composite Particles&gt;

20 kg of spherical magnetite particles shown in the electron micrograph ( $\times 20,000$ ) of FIG. 1 (average particle size: 0.23  $\mu\text{m}$ ; geometrical standard deviation value: 1.42; BET specific surface area value: 9.2  $\text{m}^2/\text{g}$ ; blackness (L\* value): 20.6; fluidity index: 35; coercive force value: 61 Oe; saturation magnetization value in a magnetic field of 10 kOe: 84.9 emu/g; residual magnetization value in a magnetic field of 10 kOe: 7.8 emu/g), were deagglomerated in 150 liters of pure water using a stirrer, and further passed through a "TK pipeline homomixer" (tradename, manufactured by Tokushu Kika Kogyo Co., Ltd.) three times, thereby obtaining a slurry containing the spherical magnetite particles.

Successively, the obtained slurry containing the spherical magnetite particles was passed through a transverse-type sand grinder (tradename "MIGHTY MILL MHG-1.5L", manufactured by Inoue Seisakusho Co., Ltd.) five times at an axis-rotating speed of 2,000 rpm, thereby obtaining a slurry in which the spherical magnetite particles were dispersed.

The particles in the obtained slurry which remained on a sieve of 325 meshes (mesh size: 44  $\mu\text{m}$ ) was 0%. The slurry was filtered and washed with water, thereby obtaining a filter cake containing the spherical magnetite particles. After the obtained filter cake containing the spherical magnetite particles was dried at 120° C., 11.0 kg of the dried particles were then charged into an edge runner "MPUV-2 Model" (tradename, manufactured by Matsumoto Chuzo Tekkoshou Co., Ltd.), and mixed and stirred at 30 Kg/cm and a stirring speed of 22 rpm for 30 minutes, thereby lightly deagglomerating the particles.

110 g of methyl hydrogen polysiloxane (tradename: "TSF484", produced by TOSHIBA SILICONE CO., LTD.) were added to the deagglomerated spherical magnetite particles under the operation of the edge runner. The spherical magnetite particles were continuously mixed and stirred at a linear load of 60 Kg/cm and a stirring speed of 22 rpm for 60 minutes to form a coating layer composed of methyl hydrogen polysiloxane on the spherical magnetite particles..

Next, 990 g of carbon black fine particles shown in the electron micrograph ( $\times 20,000$ ) of FIG. 2 (particle shape: granular shape; average particle size: 0.022  $\mu\text{m}$ ; geometrical standard deviation value: 1.68; BET specific surface area value: 134  $\text{m}^2/\text{g}$ ; and blackness (L\* value): 16.6) were added to the spherical magnetite particles coated with methyl hydrogen polysiloxane for 10 minutes while operating the edge runner. Further, the mixed particles were continuously stirred at a linear load of 60 Kg/cm and a stirring speed of 22 rpm for 60 minutes to form the carbon black coat on the coating layer composed of methyl hydrogen polysiloxane, thereby obtaining black magnetic composite particles.

The obtained black magnetic composite particles were dried at 105° C. for 60 minutes by using a drier to evaporate water or the like which were remained on surfaces of the composite particles. The obtained black magnetic composite particles had an average particle size of 0.24  $\mu\text{m}$ . In addition, the black magnetic composite particles had a geometrical standard deviation value of 1.42, a BET specific surface area value of 9.8  $\text{m}^2/\text{g}$ , a fluidity index of 48 and a blackness (L\* value) of 18.2. The desorption percentage of the carbon black from the black magnetic composite particles was 6.5%. As to the magnetic properties, the coercive force value of the black magnetic composite particles was 59 Oe; the saturation magnetization value in a magnetic field of 10 kOe was 76.8 emu/g; and the residual magnetization value in a magnetic field of 10 kOe was 7.0 emu/g. The coating amount of methyl hydrogen polysiloxane was 0.44% by weight calculated as Si. The amount of the carbon black coat formed on the coating layer composed of methyl hydrogen polysiloxane is 8.21% by weight (calculated as C) based on the weight of the black magnetic composite particles (corresponding to 9 parts by weight based on 100 parts by weight of the spherical magnetite particles). The thickness of the carbon black coat formed was 0.0024  $\mu\text{m}$ . Since no independent carbon black was observed on the electron micrograph, it was confirmed that a whole amount of the carbon black used contributed to the formation of the carbon black coat on the coating layer composed of methyl hydrogen polysiloxane.

## Example 4

## &lt;Production of Black Magnetic Toner Containing Black Magnetic Composite Particles&gt;

400 g of the black magnetic composite particles obtained in Example 3, 540 g of styrene-butyl acrylate-methyl methacrylate copolymer resin (molecular weight=130,000, styrene/butyl acrylate/methyl methacrylate =82.0/16.5/1.5), 60 g of polypropylene wax (molecular weight: 3,000) and 15

g of a charge-controlling agent were charged into a Henschel mixer, and mixed and stirred therein at 60° C. for 15 minutes. The obtained mixed particles were melt-kneaded at 140° C. using a continuous-type twin-screw kneader (T-1), and the obtained kneaded material was cooled, coarsely pulverized and finely pulverized in air. The obtained particles were subjected to classification, thereby producing a black magnetic toner.

The obtained black magnetic toner had an average particle size of 9.7  $\mu\text{m}$ , a dispersibility of 5th rank, a fluidity index of 72, a blackness (L\* value) of 18.1, a volume resistivity of  $1.2 \times 10^{14} \Omega\text{-cm}$ , a coercive force value of 59 Oe, a saturation magnetization value (in a magnetic field of 10 kOe) of 32.4 emu/g, a residual magnetization value (in a magnetic field of 10 kOe) of 4.1 emu/g, a saturation magnetization value (in a magnetic field of 1 kOe) of 25.7 emu/g, and a residual magnetization value (in a magnetic field of 1 kOe) of 3.4 emu/g.

#### Example 5

##### <Production of Black Magnetic Composite Particles>

20 kg of spherical magnetite particles shown in the electron micrograph ( $\times 20,000$ ) of FIG. 1 (average particle size: 0.23  $\mu\text{m}$ ; geometrical standard deviation value: 1.42; BET specific surface area value: 9.2  $\text{m}^2/\text{g}$ ; blackness (L\* value): 20.6; fluidity index: 35; coercive force value: 61 Oe; saturation magnetization value in a magnetic field of 10 kOe: 84.9 emu/g; residual magnetization value in a magnetic field of 10 kOe: 7.8 emu/g), were deagglomerated in 150 liters of pure water using a stirrer, and further passed through a "TK pipeline homomixer" (tradename, manufactured by Tokushu Kika Kogyo Co., Ltd.) three times, thereby obtaining a slurry containing the spherical magnetite particles.

Successively, the obtained slurry containing the spherical magnetite particles was passed through a transverse-type sand grinder (tradename "MIGHTY MILL MHG-1.5L", manufactured by Inoue Seisakusho Co., Ltd.) five times at an axis-rotating speed of 2,000 rpm, thereby obtaining a slurry in which the spherical magnetite particles were dispersed.

The particles in the obtained slurry which remained on a sieve of 325 meshes (mesh size: 44  $\mu\text{m}$ ) was 0%. The slurry was filtered and washed with water, thereby obtaining a filter cake containing the spherical magnetite particles. After the obtained filter cake containing the spherical magnetite particles was dried at 120° C., 11.0 kg of the dried particles were then charged into an edge runner "MPUV-2 Model" (tradename, manufactured by Matsumoto Chuzo Tekkosho Co., Ltd.), and mixed and stirred at 30 Kg/cm and a stirring speed of 22 rpm for 30 minutes, thereby lightly deagglomerating the particles.

220 g of tridecafluoroctyl trimethoxysilane (tradename "TSL8257", produced by TOSHIBA SILICONE CO., LTD.) were added to the deagglomerated spherical magnetite particles under the operation of the edge runner. The spherical magnetite particles were continuously mixed and stirred at a linear load of 60 Kg/cm and a stirring speed of 22 rpm for 60 minutes to form a coating layer composed of tridecafluoroctyl trimethoxysilane on the surface of the black manganese-containing hematite particles.

Next, 990 g of carbon black fine particles shown in the electron micrograph ( $\times 20,000$ ) of FIG. 2 (particle shape: granular shape; average particle size: 0.022  $\mu\text{m}$ ; geometrical standard deviation value: 1.68; BET specific surface area value: 134  $\text{m}^2/\text{g}$ ; and blackness (L\* value): 16.6) were added to the spherical magnetite particles coated with tridecafluoroctyl trimethoxysilane for 10 minutes while operating the edge runner. Further, the mixed particles were continuously

stirred at a linear load of 60 Kg/cm and a stirring speed of 22 rpm for 60 minutes to form the carbon black coat on the coating layer composed of tridecafluoroctyl trimethoxysilane, thereby obtaining black magnetic composite particles.

The obtained black magnetic composite particles were heat-treated at 105° C. for 60 minutes by using a drier to evaporate water or the like which were remained on surfaces of the composite particles. The obtained black magnetic composite particles had an average particle size of 0.24  $\mu\text{m}$ . In addition, the black magnetic composite particles showed a geometrical standard deviation value of 1.42, a BET specific surface area value of 8.6  $\text{m}^2/\text{g}$ , a fluidity index of 48 and a blackness (L\* value) of 18.4. The desorption percentage of the carbon black from the black magnetic composite particles was 6.8%. As to the magnetic properties, the coercive force value of the black magnetic composite particles was 61 Oe; the saturation magnetization value in a magnetic field of 10 kOe was 76.8 emu/g; and the residual magnetization value in a magnetic field of 10 kOe was 6.9 emu/g. The amount of a coating layer composed of a fluorine-containing organosilane compound produced from tridecafluoroctyl trimethoxysilane was 0.13% by weight calculated as Si. The amount of the carbon black coat formed on the coating layer composed of the fluoroalkyl organosilane compound produced from tridecafluoroctyl trimethoxysilane is 8.15% by weight (calculated as C) based on the weight of the black magnetic composite particles (corresponding to 9 parts by weight based on 100 parts by weight of the spherical magnetite particles). The thickness of the carbon black coat formed was 0.0024  $\mu\text{m}$ . Since no independent carbon black was observed on the electron micrograph, it was confirmed that a whole amount of the carbon black used contributed to the formation of the carbon black coat on the coating layer composed of the fluorine-containing organosilane compound produced from tridecafluoroctyl trimethoxysilane.

#### Example 6

##### <Production of Black Magnetic Toner Containing Black Magnetic Composite Particles>

400 g of the black magnetic composite particles obtained in Example 5, 540 g of styrene-butyl acrylate-methyl methacrylate copolymer resin (molecular weight=130,000, styrene/butyl acrylate/methyl methacrylate =82.0/16.5/1.5), 60 g of polypropylene wax (molecular weight: 3,000) and 15 g of a charge-controlling agent were charged into a Henschel mixer, and mixed and stirred therein at 60° C. for 15 minutes. The obtained mixed particles were melt-kneaded at 140° C. using a continuous-type twin-screw kneader (T-1), and the obtained kneaded material was cooled, coarsely pulverized and finely pulverized in air. The obtained particles were subjected to classification, thereby producing a black magnetic toner.

The obtained black magnetic toner had an average particle size of 10.1  $\mu\text{m}$ , a dispersibility of 5th rank, a fluidity index of 75, a blackness (L\* value) of 18.5, a volume resistivity of  $1.3 \times 10^{14} \Omega\text{-cm}$ , a coercive force value of 58 Oe, a saturation magnetization value (in a magnetic field of 10 kOe) of 32.4 emu/g, a residual magnetization value (in a magnetic field of 10 kOe) of 4.2 emu/g, a saturation magnetization value (in a magnetic field of 1 kOe) of 25.7 emu/g, and a residual magnetization value (in a magnetic field of 1 kOe) of 3.4 emu/g.

#### Core Particles 1 to 4

Various magnetic iron oxide particles were prepared by known methods. The same procedure as defined in Example 1 was conducted by using the thus prepared particles,

thereby obtaining deagglomerated magnetic iron oxide particles as core particles.

Various properties of the thus obtained magnetic iron oxide particles are shown in Table 1.

#### Core Particles 5

The same procedure as defined in Example 1 was conducted by using 20 kg of the deagglomerated octahedral magnetite particles (core particles 1) and 150 liters of water, thereby obtaining a slurry containing the octahedral magnetite particles. The pH value of the obtained re-dispersed slurry containing the octahedral magnetite particles was adjusted to 4.0, and then the concentration of the slurry was adjusted to 98 g/liter by adding water thereto. After 150 liters of the slurry was heated to 60° C., 2722 ml of a 1.0 mol/liter aluminum sulfate solution (equivalent to 1.0% by weight (calculated as Al) based on the weight of the octahedral magnetite particles) was added to the slurry. After allowing the slurry to stand for 30 minutes, the pH value of the slurry was adjusted to 7.5 by adding an aqueous sodium hydroxide solution. Successively, 254 g of water glass #3 (equivalent to 0.5% by weight (calculated as SiO<sub>2</sub>) based on the weight of the octahedral magnetite particles) was added to the slurry. After the slurry was aged for 30 minutes, the pH value of the slurry was adjusted to 7.5 by adding acetic acid. After further allowing the slurry to stand for 30 minutes, the slurry was subjected to filtration, washing with water, drying and pulverization, thereby obtaining the octahedral magnetite particles coated with hydroxides of aluminum and oxides of silicon.

Main production conditions are shown in Table 2, and various properties of the obtained octahedral magnetite particles are shown in Table 3.

#### Core Particles 6 to 8

The same procedure as defined in the production of the core particles 5 above, was conducted except that kind of core particles, and kind and amount of additives used in the surface treatment were varied, thereby obtaining surface-treated magnetic iron oxide particles.

Main production conditions are shown in Table 2, and various properties of the obtained surface-treated magnetic iron oxide particles are shown in Table 3.

#### Examples 7 to 14 and Comparative Examples 1 to 5

The same procedure as defined in Example 1 was conducted except that kind of particles to be treated, addition or non-addition of an alkoxysilane compound in the coating treatment with alkoxysilane compound, kind and amount of the alkoxysilane compound added, treating conditions of edge runner in the coating treatment, kind and amount of carbon black coat formed, and treating conditions of edge runner used in the process for forming the carbon black coat, were varied, thereby obtaining black magnetic composite particles. The black magnetic composite particles obtained in Examples 7 to 14 were observed by an electron microscope. As a result, almost no independent carbon black was recognized. Therefore, it was confirmed that a substantially whole amount of the carbon black contributed to the formation of the carbon black coat on the coating layer composed of organosilane compound produced from the alkoxysilane compound.

Various properties of the carbon black fine particles A to C are shown in Table 4.

Main production conditions are shown in Table 5, and various properties of the obtained black magnetic composite particles are shown in Table 6.

Meanwhile, in Comparative Example 1, the spherical magnetite particles uncoated with the alkoxysilane com-

pound and the carbon black fine particles were mixed and stirred together by an edge runner in the same manner as described above, thereby obtaining treated particles. An electron micrograph (×20,000) of the thus treated particles is shown in FIG. 4. As shown in FIG. 4, it was confirmed that the carbon black was not adhered on the surfaces of the spherical magnetite particles, and both the particles were present independently.

#### Examples 15 to 22 and Comparative Examples 6 to 14

##### <Production of Black Magnetic Toner>

The same procedure as defined in Example 2 was conducted by using the black magnetic composite particles obtained in Examples 7 to 14, the magnetic iron oxide particles as core particles 1 to 4, the mixed particles composed of the magnetic iron oxide particles and the carbon black fine particles used in Comparative Example 1 and the black magnetic composite particles obtained in Comparative Examples 2 to 5, thereby obtaining black magnetic toners.

Main production conditions and various properties of the obtained black magnetic toners are shown in Tables 7 and 8.

#### Examples 23 to 46 and Comparative Examples 15 to 23

The same procedure as defined in Example 3 was conducted except that kind of particles to be treated, addition or non-addition of a polysiloxane or modified polysiloxane, kind and amount of the polysiloxane or modified polysiloxane, treating conditions of edge runner in the coating treatment, kind and amount of carbon black coat formed, and treating conditions of edge runner used in the process for forming the carbon black coat, were varied, thereby obtaining black magnetic composite particles. The black magnetic composite particles obtained in Examples 23 to 46 were observed by an electron microscope. As a result, almost no independent carbon black was recognized. Therefore, it was confirmed that a substantially whole amount of the carbon black contributed to the formation of the carbon black coat on the coating layer composed of polysiloxane or modified polysiloxane.

Main production conditions are shown in Tables 9 to 11, and various properties of the obtained black magnetic composite particles are shown in Tables 12 to 14.

#### Examples 47 to 70 and Comparative Examples 24 to 32

##### <Production of Black Magnetic Toner>

The same procedure as defined in Example 4 was conducted by using the black magnetic composite particles obtained in Examples 47 to 70, and the black magnetic composite particles obtained in Comparative Examples 15 to 23, thereby obtaining black magnetic toners.

Main production conditions and various properties of the obtained black magnetic toners are shown in Tables 15 to 17.

#### Examples 71 to 78 and Comparative Examples 33 to 35

The same procedure as defined in Example 5 was conducted except that kind of particles to be treated, addition or non-addition of a fluoroalkyl organosilane compound, kind and amount of the fluoroalkyl organosilane compound added, treating conditions of edge runner in the coating treatment, kind and amount of carbon black coat formed, and treating conditions of edge runner used in the process for forming the carbon black coat, were varied, thereby obtain-

ing black magnetic composite particles. The black magnetic composite particles obtained in Examples 71 to 78 were observed by an electron microscope. As a result, almost no independent carbon black was recognized. Therefore, it was confirmed that a substantially whole amount of the carbon black contributed to the formation of the carbon black coat on the coating layer composed of a fluorine-containing organosilane compound produced from the fluoroalkyl organosilane compound.

Main production conditions are shown in Table 18, and various properties of the obtained black magnetic composite particles are shown in Table 19.

Examples 79 to 86 and Comparative Examples 36 to 38

<Production of Black Magnetic Toner>

The same procedure as defined in Example 6 was conducted by using the black magnetic composite particles obtained in Examples 71 to 78, and the black magnetic composite particles obtained in Comparative Examples 33 to 35, thereby obtaining black magnetic toners.

Main production conditions and various properties of the obtained black magnetic toners are shown in Table 20.

TABLE 1

| Properties of magnetic iron oxide particles |                     |                |                                         |                  |                                    |
|---------------------------------------------|---------------------|----------------|-----------------------------------------|------------------|------------------------------------|
| Core particles                              | Kind                | Particle shape | Average particle size ( $\mu\text{m}$ ) | Aspect ratio (-) | Geometrical standard deviation (-) |
| Core particles 1                            | Magnetite particles | Octahedral     | 0.28                                    | —                | 1.53                               |
| Core particles 2                            | Magnetite particles | Spherical      | 0.23                                    | —                | 1.35                               |
| Core particles 3                            | Magnetite particles | Acicular       | 0.40                                    | 8.1:1            | 1.53                               |
| Core particles 4                            | Maghemite particles | Spherical      | 0.20                                    | —                | 1.42                               |

| Properties of magnetic iron oxide particles |                                                     |                     |                                           |                                         |                    |
|---------------------------------------------|-----------------------------------------------------|---------------------|-------------------------------------------|-----------------------------------------|--------------------|
| Magnetic properties                         |                                                     |                     |                                           |                                         |                    |
| Core particles                              | BET specific surface area ( $\text{m}^2/\text{g}$ ) | Coercive force (Oe) | Saturation magnetization (10 kOe) (emu/g) | Residual magnetization (10 kOe) (emu/g) | Fluidity index (-) |
| Core particles 1                            | 4.6                                                 | 101                 | 86.8                                      | 12.2                                    | 34                 |
| Core particles 2                            | 11.8                                                | 63                  | 85.1                                      | 7.7                                     | 38                 |
| Core particles 3                            | 18.8                                                | 343                 | 86.3                                      | 29.3                                    | 32                 |
| Core particles 4                            | 7.2                                                 | 54                  | 78.8                                      | 8.7                                     | 38                 |
|                                             |                                                     |                     |                                           |                                         | 31.5               |

TABLE 2

| Core particles   | Kind of core particles | Surface-treating process Additives   |                        |                |
|------------------|------------------------|--------------------------------------|------------------------|----------------|
|                  |                        | Kind                                 | Calculated as          | Amount (wt. %) |
| Core particles 5 | Core particles 1       | Aluminum sulfate<br>Water glass #3   | Al<br>SiO <sub>2</sub> | 1.0<br>0.5     |
| Core particles 6 | Core particles 2       | Sodium aluminate<br>Colloidal silica | Al<br>SiO <sub>2</sub> | 2.0<br>1.0     |
| Core particles 7 | Core particles 3       | Aluminum acetate                     | Al                     | 5.0            |
| Core particles 8 | Core particles 4       | Water glass #3                       | SiO <sub>2</sub>       | 1.0            |

  

| Core particles   | Surface-treating process Coating material |                  |                |
|------------------|-------------------------------------------|------------------|----------------|
|                  | Kind                                      | Calculated as    | Amount (wt. %) |
| Core particles 5 | A                                         | Al               | 0.98           |
|                  | S                                         | SiO <sub>2</sub> | 0.49           |
| Core particles 6 | A                                         | Al               | 1.92           |
|                  | S                                         | SiO <sub>2</sub> | 0.96           |
| Core particles 7 | A                                         | Al               | 4.75           |
| Core particles 8 | S                                         | SiO <sub>2</sub> | 0.98           |

Note; A: Hydroxide of aluminum

S: Oxide of silicon

TABLE 3

| Core particles   | Properties of surface-treated magnetic iron oxide particles |                  |                                    |                                                     |  |
|------------------|-------------------------------------------------------------|------------------|------------------------------------|-----------------------------------------------------|--|
|                  | Average particle size ( $\mu\text{m}$ )                     | Aspect ratio (-) | Geometrical standard deviation (-) | BET specific surface area ( $\text{m}^2/\text{g}$ ) |  |
| Core particles 5 | 0.29                                                        | —                | 1.51                               | 9.8                                                 |  |
| Core particles 6 | 0.24                                                        | —                | 1.35                               | 13.6                                                |  |
| Core particles 7 | 0.40                                                        | 8.1:1            | 1.52                               | 25.4                                                |  |
| Core particles 8 | 0.20                                                        | —                | 1.42                               | 7.5                                                 |  |

  

| Properties of surface-treated magnetic iron oxide particles |                     |                                           |                                         |                    |                              |
|-------------------------------------------------------------|---------------------|-------------------------------------------|-----------------------------------------|--------------------|------------------------------|
| Magnetic properties                                         |                     |                                           |                                         |                    |                              |
| Core particles                                              | Coercive force (Oe) | Saturation magnetization (10 kOe) (emu/g) | Residual magnetization (10 kOe) (emu/g) | Fluidity index (-) | Blackness ( $L^*$ value) (-) |
| Core particles 5                                            | 103                 | 86.3                                      | 12.1                                    | 32                 | 21.4                         |

TABLE 3-continued

|                  |     |      |      |    |      |
|------------------|-----|------|------|----|------|
| Core particles 6 | 62  | 84.8 | 7.6  | 37 | 20.8 |
| Core particles 7 | 336 | 86.0 | 19.8 | 32 | 24.6 |
| Core particles 8 | 53  | 78.6 | 8.6  | 37 | 31.6 |

TABLE 4

| Properties of carbon black fine particles |                |                                         |                                    |
|-------------------------------------------|----------------|-----------------------------------------|------------------------------------|
| Kind of carbon black fine particles       | Particle shape | Average particle size ( $\mu\text{m}$ ) | Geometrical standard deviation (-) |
| Carbon black A                            | Granular       | 0.022                                   | 1.78                               |
| Carbon black B                            | Granular       | 0.015                                   | 1.56                               |
| Carbon black C                            | Granular       | 0.030                                   | 2.06                               |

  

| Properties of carbon black fine particles |                                                     |                              |
|-------------------------------------------|-----------------------------------------------------|------------------------------|
| Kind of carbon black fine particles       | BET specific surface area ( $\text{m}^2/\text{g}$ ) | Blackness ( $L^*$ value) (-) |
| Carbon black A                            | 133.5                                               | 14.6                         |
| Carbon black B                            | 265.3                                               | 15.2                         |
| Carbon black C                            | 84.6                                                | 17.0                         |

TABLE 5

| Production of black magnetic composite particles    |                                  |                           |                               |
|-----------------------------------------------------|----------------------------------|---------------------------|-------------------------------|
| Coating step with alkoxy silane or silicon compound |                                  |                           |                               |
| Alkoxy silane compound                              |                                  |                           |                               |
| Examples and Comparative Examples                   | Kind of particles to be treated  | Kind                      | Amount added (part by weight) |
| Example 7                                           | Core particles 1                 | Dimethyl dimethoxysilane  | 1.0                           |
| Example 8                                           | Core particles 2                 | Phenyl triethoxysilane    | 0.5                           |
| Example 9                                           | Core particles 3                 | Isobutyl trimethoxysilane | 5.0                           |
| Example 10                                          | Core particles 4                 | Methyl triethoxysilane    | 1.5                           |
| Example 11                                          | Core particles 5                 | Dimethyl dimethoxysilane  | 0.2                           |
| Example 12                                          | Core particles 6                 | Phenyl triethoxysilane    | 1.5                           |
| Example 13                                          | Core particles 7                 | Isobutyl trimethoxysilane | 1.0                           |
| Example 14                                          | Core particles 8                 | Methyl triethoxysilane    | 2.0                           |
| Comparative Example 1                               | Core particles used in Example 1 | —                         | —                             |
| Comparative Example 2                               | Core particles 1                 | Methyl triethoxysilane    | 1.0                           |
| Comparative Example 3                               | Core particles 1                 | Dimethyl dimethoxysilane  | 0.5                           |
| Comparative Example 4                               | Core particles 1                 | Methyl triethoxysilane    | 0.005                         |

TABLE 5-continued

| Comparative Example 5                               | Core particles 1                              | $\gamma$ -aminopropyl triethoxysilane | 1.0                  |
|-----------------------------------------------------|-----------------------------------------------|---------------------------------------|----------------------|
| Production of black magnetic composite particles    |                                               |                                       |                      |
| Coating step with alkoxy silane or silicon compound |                                               |                                       |                      |
| Examples and                                        | Edge runner treatment                         | Coating amount (calculated as         |                      |
| Comparative Examples                                | Linear load (Kg/cm)                           | Time (min)                            | Si (wt. %)           |
| Example 7                                           | 45                                            | 15                                    | 0.22                 |
| Example 8                                           | 75                                            | 20                                    | 0.06                 |
| Example 9                                           | 30                                            | 60                                    | 0.73                 |
| Example 10                                          | 60                                            | 30                                    | 0.24                 |
| Example 11                                          | 60                                            | 20                                    | 0.05                 |
| Example 12                                          | 30                                            | 60                                    | 0.18                 |
| Example 13                                          | 45                                            | 30                                    | 0.16                 |
| Example 14                                          | 60                                            | 30                                    | 0.32                 |
| Comparative Example 1                               | —                                             | —                                     | —                    |
| Comparative Example 2                               | 30                                            | 60                                    | 0.21                 |
| Comparative Example 3                               | 60                                            | 30                                    | 0.11                 |
| Comparative Example 4                               | 60                                            | 30                                    | $7.9 \times 10^{-4}$ |
| Comparative Example 5                               | 60                                            | 60                                    | 0.126                |
| Production of black magnetic composite particles    |                                               |                                       |                      |
| Adhering step of carbon black                       |                                               |                                       |                      |
| Carbon black fine particles                         |                                               |                                       |                      |
| Examples and                                        | Kind                                          | Amount added (part by weight)         |                      |
| Comparative Examples                                | Kind                                          | Amount added (part by weight)         |                      |
| Example 7                                           | B                                             | 6.0                                   |                      |
| Example 8                                           | B                                             | 12.0                                  |                      |
| Example 9                                           | C                                             | 16.0                                  |                      |
| Example 10                                          | A                                             | 25.0                                  |                      |
| Example 11                                          | B                                             | 20.0                                  |                      |
| Example 12                                          | B                                             | 15.0                                  |                      |
| Example 13                                          | C                                             | 10.0                                  |                      |
| Example 14                                          | A                                             | 20.0                                  |                      |
| Comparative Example 1                               | Carbon black fine particles used in Example 1 | 10.0                                  |                      |
| Comparative Example 2                               | —                                             | —                                     |                      |
| Comparative Example 3                               | A                                             | 0.01                                  |                      |
| Comparative Example 4                               | B                                             | 5.0                                   |                      |
| Comparative Example 5                               | C                                             | 7.0                                   |                      |
| Production of black magnetic composite particles    |                                               |                                       |                      |
| Adhering step of carbon black                       |                                               |                                       |                      |
| Examples and                                        | Edge runner treatment                         | Amount adhered (calculated as C)      |                      |
| Comparative Examples                                | Linear load (Kg/cm)                           | Time (min)                            | (wt. %)              |
| Example 7                                           | 30                                            | 60                                    | 5.66                 |
| Example 8                                           | 30                                            | 90                                    | 10.73                |
| Example 9                                           | 45                                            | 45                                    | 13.70                |
| Example 10                                          | 60                                            | 60                                    | 22.65                |
| Example 11                                          | 30                                            | 45                                    | 16.63                |
| Example 12                                          | 60                                            | 60                                    | 12.99                |
| Example 13                                          | 60                                            | 30                                    | 9.09                 |
| Example 14                                          | 75                                            | 30                                    | 17.09                |

TABLE 5-continued

|                       |    |    |      |
|-----------------------|----|----|------|
| Comparative Example 1 | 60 | 30 | 9.06 |
| Comparative Example 2 | —  | —  | —    |
| Comparative Example 3 | 30 | 60 | 0.01 |
| Comparative Example 4 | 60 | 45 | 4.75 |
| Comparative Example 5 | 60 | 30 | 2.88 |

TABLE 6

| Examples and Comparative Examples | Properties of black magnetic composite particles |                  |                                    |                                                     |
|-----------------------------------|--------------------------------------------------|------------------|------------------------------------|-----------------------------------------------------|
|                                   | Average particle size ( $\mu\text{m}$ )          | Aspect ratio (-) | Geometrical standard deviation (-) | BET specific surface area ( $\text{m}^2/\text{g}$ ) |
| Example 7                         | 0.28                                             | —                | 1.52                               | 5.0                                                 |
| Example 8                         | 0.24                                             | —                | 1.34                               | 13.6                                                |
| Example 9                         | 0.41                                             | 8.1:1            | 1.51                               | 23.8                                                |
| Example 10                        | 0.23                                             | —                | 1.43                               | 15.3                                                |
| Example 11                        | 0.30                                             | —                | 1.47                               | 14.4                                                |
| Example 12                        | 0.24                                             | —                | 1.34                               | 16.1                                                |
| Example 13                        | 0.40                                             | 8.0:1            | 1.50                               | 24.8                                                |
| Example 14                        | 0.23                                             | —                | 1.42                               | 13.8                                                |
| Comparative Example 1             | 0.29                                             | —                | 1.53                               | 11.9                                                |
| Comparative Example 2             | 0.29                                             | —                | 1.52                               | 10.6                                                |
| Comparative Example 3             | 0.28                                             | —                | 1.52                               | 5.6                                                 |
| Comparative Example 4             | 0.28                                             | —                | 1.52                               | 17.6                                                |
| Comparative Example 5             | 0.29                                             | —                | 1.52                               | 11.2                                                |

Properties of black magnetic composite particles

Magnetic properties

| Examples and Comparative Examples | Coercive force (Oe) | Saturation magnetization (10 kOe) (emu/g) | Residual magnetization (10 kOe) (emu/g) | Examples | Example 19 | Example 11 | 45 |
|-----------------------------------|---------------------|-------------------------------------------|-----------------------------------------|----------|------------|------------|----|
|                                   |                     |                                           |                                         |          |            |            |    |
| Example 7                         | 108                 | 81.1                                      | 11.4                                    |          |            |            |    |
| Example 8                         | 65                  | 71.8                                      | 6.5                                     |          |            |            |    |
| Example 9                         | 336                 | 73.8                                      | 25.8                                    |          |            |            |    |
| Example 10                        | 58                  | 63.6                                      | 6.4                                     |          |            |            |    |
| Example 11                        | 106                 | 72.8                                      | 10.2                                    |          |            |            |    |
| Example 12                        | 68                  | 74.1                                      | 6.7                                     |          |            |            |    |
| Example 13                        | 331                 | 77.8                                      | 27.2                                    |          |            |            |    |
| Example 14                        | 57                  | 65.6                                      | 7.2                                     |          |            |            |    |
| Comparative Example 1             | 103                 | 79.3                                      | 10.3                                    |          |            |            |    |
| Comparative Example 2             | 103                 | 83.6                                      | 10.8                                    |          |            |            |    |
| Comparative Example 3             | 104                 | 86.7                                      | 11.3                                    |          |            |            |    |
| Comparative Example 4             | 100                 | 83.8                                      | 10.9                                    |          |            |            |    |
| Comparative Example 5             | 102                 | 84.6                                      | 10.6                                    |          |            |            |    |

TABLE 6-continued

| Examples and Comparative Examples | Fluidity index (-) | Blackness ( $L^*$ value) (-) | Properties of black magnetic composite particles |                                                  |
|-----------------------------------|--------------------|------------------------------|--------------------------------------------------|--------------------------------------------------|
|                                   |                    |                              | Carbon black desorption percentage (%)           | Thickness of carbon black coat ( $\mu\text{m}$ ) |
| Example 7                         | 49                 | 17.0                         | 8.6                                              | 0.0023                                           |
| Example 8                         | 45                 | 16.4                         | 8.2                                              | 0.0024                                           |
| Example 9                         | 46                 | 17.8                         | 6.4                                              | 0.0026                                           |
| Example 10                        | 54                 | 17.5                         | 5.2                                              | 0.0027                                           |
| Example 11                        | 52                 | 15.9                         | 3.1                                              | 0.0027                                           |
| Example 12                        | 47                 | 16.2                         | 3.6                                              | 0.0025                                           |
| Example 13                        | 48                 | 17.5                         | 2.1                                              | 0.0024                                           |
| Example 14                        | 51                 | 17.9                         | 3.8                                              | 0.0026                                           |
| Comparative Example 1             | 42                 | 20.0                         | 78.6                                             | —                                                |
| Comparative Example 2             | 40                 | 20.9                         | —                                                | —                                                |
| Comparative Example 3             | 38                 | 21.4                         | 31.2                                             | —                                                |
| Comparative Example 4             | 40                 | 20.1                         | 26.5                                             | —                                                |
| Comparative Example 5             | 41                 | 20.6                         | 41.6                                             | —                                                |

  

| TABLE 7                            |            |                                 |                               |                                 |
|------------------------------------|------------|---------------------------------|-------------------------------|---------------------------------|
| Production of black magnetic toner |            |                                 |                               |                                 |
| Black magnetic composite particles |            | Resin                           |                               |                                 |
| Examples                           | Kind       | Amount blended (part by weight) | Kind                          | Amount blended (part by weight) |
| Example 15                         | Example 7  | 45                              | Styrene-acryl copolymer resin | 55                              |
| Example 16                         | Example 8  | 45                              | Styrene-acryl copolymer resin | 55                              |
| Example 17                         | Example 9  | 40                              | Styrene-acryl copolymer resin | 60                              |
| Example 18                         | Example 10 | 50                              | Styrene-acryl copolymer resin | 50                              |
| Example 19                         | Example 11 | 45                              | Styrene-acryl copolymer resin | 55                              |
| Example 20                         | Example 12 | 40                              | Styrene-acryl copolymer resin | 60                              |
| Example 21                         | Example 13 | 50                              | Styrene-acryl copolymer resin | 50                              |
| Example 22                         | Example 14 | 50                              | Styrene-acryl copolymer resin | 50                              |

  

| Properties of black magnetic toner |                                         |                    |                    |                                                 |
|------------------------------------|-----------------------------------------|--------------------|--------------------|-------------------------------------------------|
| Examples                           | Average particle size ( $\mu\text{m}$ ) | Dispersibility (-) | Fluidity index (-) | Volume resistivity ( $\Omega \cdot \text{cm}$ ) |
|                                    |                                         |                    |                    |                                                 |
| Example 15                         | 9.6                                     | 4                  | 74                 | $9.8 \times 10^{13}$                            |
| Example 16                         | 10.1                                    | 5                  | 82                 | $1.6 \times 10^{14}$                            |
| Example 17                         | 11.2                                    | 4                  | 72                 | $7.3 \times 10^{13}$                            |
| Example 18                         | 10.6                                    | 5                  | 78                 | $8.6 \times 10^{13}$                            |

TABLE 7-continued

|                                    |      |                          |                  |                      |                |
|------------------------------------|------|--------------------------|------------------|----------------------|----------------|
| Example 19                         | 9.2  | 5                        | 78               | $6.8 \times 10^{13}$ | 5              |
| Example 20                         | 9.8  | 5                        | 86               | $2.6 \times 10^{14}$ |                |
| Example 21                         | 8.9  | 5                        | 73               | $1.8 \times 10^{14}$ |                |
| Example 22                         | 11.0 | 5                        | 82               | $1.1 \times 10^{14}$ |                |
| Properties of black magnetic toner |      |                          |                  |                      |                |
| Magnetic properties                |      |                          |                  |                      |                |
| Coercive                           |      | Saturation magnetization |                  | 10                   |                |
| Examples                           |      | force (Oe)               | (10 kOe) (emu/g) | (1 kOe) (emu/g)      |                |
| Example 15                         | 96   | 36.8                     | 27.6             | 15                   |                |
| Example 16                         | 61   | 33.6                     | 26.1             |                      |                |
| Example 17                         | 311  | 31.4                     | 23.4             |                      |                |
| Example 18                         | 56   | 32.3                     | 22.7             |                      |                |
| Example 19                         | 103  | 32.3                     | 23.6             |                      |                |
| Example 20                         | 66   | 29.6                     | 22.2             |                      |                |
| Example 21                         | 320  | 39.1                     | 29.7             |                      |                |
| Example 22                         | 53   | 31.9                     | 23.9             |                      |                |
| Properties of black magnetic toner |      |                          |                  |                      |                |
| Magnetic properties                |      |                          |                  |                      |                |
| Residual magnetization             |      | Blackness                |                  | 20                   |                |
| Examples                           |      | (10 kOe) (emu/g)         | (1 kOe) (emu/g)  |                      | (L* value) (-) |
| Example 15                         | 5.9  | 4.4                      | 18.7             |                      |                |
| Example 16                         | 4.0  | 2.9                      | 18.1             |                      |                |
| Example 17                         | 11.3 | 8.5                      | 19.6             |                      |                |
| Example 18                         | 4.5  | 3.2                      | 19.2             |                      |                |
| Example 19                         | 5.2  | 4.0                      | 17.4             |                      |                |
| Example 20                         | 3.6  | 2.7                      | 18.1             |                      |                |
| Example 21                         | 14.1 | 9.9                      | 18.9             | 25                   |                |
| Example 22                         | 4.5  | 3.1                      | 19.5             |                      |                |
| Properties of black magnetic toner |      |                          |                  |                      |                |
| Magnetic properties                |      |                          |                  |                      |                |
| Residual magnetization             |      | Blackness                |                  |                      |                |
| Examples                           |      | (10 kOe) (emu/g)         | (1 kOe) (emu/g)  |                      | (L* value) (-) |
| Example 15                         | 5.9  | 4.4                      | 18.7             |                      |                |
| Example 16                         | 4.0  | 2.9                      | 18.1             |                      |                |
| Example 17                         | 11.3 | 8.5                      | 19.6             |                      |                |
| Example 18                         | 4.5  | 3.2                      | 19.2             |                      |                |
| Example 19                         | 5.2  | 4.0                      | 17.4             | 30                   |                |
| Example 20                         | 3.6  | 2.7                      | 18.1             |                      |                |
| Example 21                         | 14.1 | 9.9                      | 18.9             |                      |                |
| Example 22                         | 4.5  | 3.1                      | 19.5             |                      |                |
| Properties of black magnetic toner |      |                          |                  |                      |                |
| Magnetic properties                |      |                          |                  |                      |                |
| Residual magnetization             |      | Blackness                |                  |                      |                |
| Examples                           |      | (10 kOe) (emu/g)         | (1 kOe) (emu/g)  |                      | (L* value) (-) |
| Example 15                         | 5.9  | 4.4                      | 18.7             |                      |                |
| Example 16                         | 4.0  | 2.9                      | 18.1             |                      |                |
| Example 17                         | 11.3 | 8.5                      | 19.6             |                      |                |
| Example 18                         | 4.5  | 3.2                      | 19.2             |                      |                |
| Example 19                         | 5.2  | 4.0                      | 17.4             | 35                   |                |
| Example 20                         | 3.6  | 2.7                      | 18.1             |                      |                |
| Example 21                         | 14.1 | 9.9                      | 18.9             |                      |                |
| Example 22                         | 4.5  | 3.1                      | 19.5             |                      |                |

TABLE 8

|                                    |                       |                                 |                               |                                 |
|------------------------------------|-----------------------|---------------------------------|-------------------------------|---------------------------------|
| Production of black magnetic toner |                       |                                 |                               |                                 |
| Black magnetic particles           |                       | Resin                           |                               | 40                              |
| Comparative Examples               | Kind                  | Amount blended (part by weight) | Kind                          | Amount blended (part by weight) |
| Comparative Example 6              | Core particles 1      | 45                              | Styrene-acryl copolymer resin | 55                              |
| Comparative Example 7              | Core particles 2      | 45                              | Styrene-acryl copolymer resin | 55                              |
| Comparative Example 8              | Core particles 3      | 45                              | Styrene-acryl copolymer resin | 55                              |
| Comparative Example 9              | Core particles 4      | 45                              | Styrene-acryl copolymer resin | 55                              |
| Comparative Example 10             | Comparative Example 1 | 45                              | Styrene-acryl copolymer resin | 55                              |
| Comparative Example 11             | Comparative Example 2 | 45                              | Styrene-acryl copolymer resin | 55                              |

TABLE 8-continued

|                                    |                        |                  |                               |                |
|------------------------------------|------------------------|------------------|-------------------------------|----------------|
| Comparative Example 12             | Comparative Example 3  | 45               | Styrene-acryl copolymer resin | 55             |
| Comparative Example 13             | Comparative Example 4  | 45               | Styrene-acryl copolymer resin | 55             |
| Comparative Example 14             | Comparative Example 5  | 45               | Styrene-acryl copolymer resin | 55             |
| Properties of black magnetic toner |                        |                  |                               |                |
| Magnetic properties                |                        |                  |                               |                |
| Residual magnetization             |                        | Blackness        |                               | 45             |
| Comparative Examples               |                        | (10 kOe) (emu/g) | (1 kOe) (emu/g)               | (L* value) (-) |
| Comparative Example 6              | Comparative Example 7  | 104              | 39.6                          | 30.0           |
| Comparative Example 7              | Comparative Example 8  | 61               | 38.8                          | 29.1           |
| Comparative Example 8              | Comparative Example 9  | 338              | 37.6                          | 28.8           |
| Comparative Example 9              | Comparative Example 10 | 51               | 34.6                          | 26.0           |
| Comparative Example 10             | Comparative Example 11 | 99               | 35.6                          | 26.3           |
| Comparative Example 11             | Comparative Example 12 | 100              | 39.1                          | 27.1           |
| Comparative Example 12             | Comparative Example 13 | 103              | 38.1                          | 29.3           |
| Comparative Example 13             | Comparative Example 14 | 102              | 36.7                          | 28.6           |
| Properties of black magnetic toner |                        |                  |                               |                |
| Magnetic properties                |                        |                  |                               |                |
| Residual magnetization             |                        | Blackness        |                               | 50             |
| Comparative Examples               |                        | (10 kOe) (emu/g) | (1 kOe) (emu/g)               | (L* value) (-) |
| Comparative Example 6              | Comparative Example 7  | 104              | 39.6                          | 30.0           |
| Comparative Example 7              | Comparative Example 8  | 61               | 38.8                          | 29.1           |
| Comparative Example 8              | Comparative Example 9  | 338              | 37.6                          | 28.8           |
| Comparative Example 9              | Comparative Example 10 | 51               | 34.6                          | 26.0           |
| Comparative Example 10             | Comparative Example 11 | 99               | 35.6                          | 26.3           |
| Comparative Example 11             | Comparative Example 12 | 100              | 39.1                          | 27.1           |
| Comparative Example 12             | Comparative Example 13 | 103              | 38.1                          | 29.3           |
| Comparative Example 13             | Comparative Example 14 | 102              | 36.7                          | 28.6           |
| Properties of black magnetic toner |                        |                  |                               |                |
| Magnetic properties                |                        |                  |                               |                |
| Residual magnetization             |                        | Blackness        |                               | 55             |
| Comparative Examples               |                        | (10 kOe) (emu/g) | (1 kOe) (emu/g)               | (L* value) (-) |
| Comparative Example 6              | Comparative Example 7  | 104              | 39.6                          | 30.0           |
| Comparative Example 7              | Comparative Example 8  | 61               | 38.8                          | 29.1           |
| Comparative Example 8              | Comparative Example 9  | 338              | 37.6                          | 28.8           |
| Comparative Example 9              | Comparative Example 10 | 51               | 34.6                          | 26.0           |
| Comparative Example 10             | Comparative Example 11 | 99               | 35.6                          | 26.3           |
| Comparative Example 11             | Comparative Example 12 | 100              | 39.1                          | 27.1           |
| Comparative Example 12             | Comparative Example 13 | 103              | 38.1                          | 29.3           |
| Comparative Example 13             | Comparative Example 14 | 102              | 36.7                          | 28.6           |
| Properties of black magnetic toner |                        |                  |                               |                |
| Magnetic properties                |                        |                  |                               |                |
| Residual magnetization             |                        | Blackness        |                               | 60             |
| Comparative Examples               |                        | (10 kOe) (emu/g) | (1 kOe) (emu/g)               | (L* value) (-) |
| Comparative Example 6              | Comparative Example 7  | 104              | 39.6                          | 30.0           |
| Comparative Example 7              | Comparative Example 8  | 61               | 38.8                          | 29.1           |
| Comparative Example 8              | Comparative Example 9  | 338              | 37.6                          | 28.8           |
| Comparative Example 9              | Comparative Example 10 | 51               | 34.6                          | 26.0           |
| Comparative Example 10             | Comparative Example 11 | 99               | 35.6                          | 26.3           |
| Comparative Example 11             | Comparative Example 12 | 100              | 39.1                          | 27.1           |
| Comparative Example 12             | Comparative Example 13 | 103              | 38.1                          | 29.3           |
| Comparative Example 13             | Comparative Example 14 | 102              | 36.7                          | 28.6           |
| Properties of black magnetic toner |                        |                  |                               |                |
| Magnetic properties                |                        |                  |                               |                |
| Residual magnetization             |                        | Blackness        |                               | 65             |
| Comparative Examples               |                        | (10 kOe) (emu/g) | (1 kOe) (emu/g)               | (L* value) (-) |
| Comparative Example 6              | Comparative Example 7  | 104              | 39.6                          | 30.0           |
| Comparative Example 7              | Comparative Example 8  | 61               | 38.8                          | 29.1           |
| Comparative Example 8              | Comparative Example 9  | 338              | 37.6                          | 28.8           |
| Comparative Example 9              | Comparative Example 10 | 51               | 34.6                          | 26.0           |
| Comparative Example 10             | Comparative Example 11 | 99               | 35.6                          | 26.3           |
| Comparative Example 11             | Comparative Example 12 | 100              | 39.1                          | 27.1           |
| Comparative Example 12             | Comparative Example 13 | 103              | 38.1                          | 29.3           |
| Comparative Example 13             | Comparative Example 14 | 102              | 36.7                          | 28.6           |

TABLE 8-continued

|                        |      |     |      |    |
|------------------------|------|-----|------|----|
| Comparative Example 8  | 12.8 | 9.7 | 26.0 |    |
| Comparative Example 9  | 3.8  | 3.0 | 34.8 | 5  |
| Comparative Example 10 | 5.0  | 3.7 | 22.6 |    |
| Comparative Example 11 | 5.9  | 4.6 | 23.3 |    |
| Comparative Example 12 | 5.3  | 4.1 | 23.5 | 10 |
| Comparative Example 13 | 5.1  | 3.9 | 22.3 |    |
| Comparative Example 14 | 4.9  | 3.8 | 22.1 | 15 |

TABLE 9

| Examples and Comparative Examples | Production of black magnetic composite particles |        |                               |
|-----------------------------------|--------------------------------------------------|--------|-------------------------------|
|                                   | Coating step with polysiloxane                   |        |                               |
|                                   | Kind of particles to be treated                  | Kind   | Amount added (part by weight) |
| Example 23                        | Core particles 1                                 | TSF484 | 1.0                           |
| Example 24                        | Core particles 2                                 | TSF484 | 5.0                           |
| Example 25                        | Core particles 3                                 | KF99   | 2.0                           |
| Example 26                        | Core particles 4                                 | L-9000 | 1.0                           |
| Example 27                        | Core particles 5                                 | TSF451 | 1.5                           |
| Example 28                        | Core particles 6                                 | TSF484 | 3.5                           |
| Example 29                        | Core particles 7                                 | KF99   | 1.0                           |
| Example 30                        | Core particles 8                                 | L-9000 | 2.0                           |
| Comparative Example 15            | Core particles 1                                 | TSF484 | 1.0                           |
| Comparative Example 16            | Core particles 1                                 | TSF484 | 0.5                           |
| Comparative Example 17            | Core particles 1                                 | TSF484 | 0.005                         |

TABLE 9

TABLE 9-continued

| Examples and Comparative Examples | Production of black magnetic composite particles |                               |  |
|-----------------------------------|--------------------------------------------------|-------------------------------|--|
|                                   | Adhering step of carbon black                    |                               |  |
|                                   | Kind                                             | Amount added (part by weight) |  |
| Example 23                        | A                                                | 10.0                          |  |
| Example 24                        | A                                                | 3.0                           |  |
| Example 25                        | B                                                | 5.0                           |  |
| Example 26                        | C                                                | 10.0                          |  |
| Example 27                        | A                                                | 5.0                           |  |
| Example 28                        | A                                                | 10.0                          |  |
| Example 29                        | B                                                | 15.0                          |  |
| Example 30                        | C                                                | 10.0                          |  |
| Comparative Example 15            | —                                                | —                             |  |
| Comparative Example 16            | A                                                | 0.01                          |  |
| Comparative Example 17            | B                                                | 3.0                           |  |

TABLE 10

| Examples and Comparative Examples | Production of black magnetic composite particles |                                   |                      |
|-----------------------------------|--------------------------------------------------|-----------------------------------|----------------------|
|                                   | Coating step with polysiloxane                   |                                   |                      |
|                                   | Edge runner treatment                            | Coating amount (calculated as Si) |                      |
| Comparative Examples              | Linear load (Kg/cm)                              | Time (min)                        | (wt. %)              |
| Example 23                        | 60                                               | 30                                | 0.44                 |
| Example 24                        | 45                                               | 25                                | 2.18                 |
| Example 25                        | 30                                               | 30                                | 0.87                 |
| Example 26                        | 60                                               | 45                                | 0.44                 |
| Example 27                        | 45                                               | 60                                | 0.62                 |
| Example 28                        | 60                                               | 30                                | 1.50                 |
| Example 29                        | 75                                               | 25                                | 0.43                 |
| Example 30                        | 60                                               | 20                                | 0.87                 |
| Comparative Example 15            | 60                                               | 30                                | 0.44                 |
| Comparative Example 16            | 60                                               | 30                                | 0.21                 |
| Comparative Example 17            | 60                                               | 30                                | $2.2 \times 10^{-3}$ |

| Examples and Comparative Examples | Production of black magnetic composite particles |         |                               |
|-----------------------------------|--------------------------------------------------|---------|-------------------------------|
|                                   | Coating step with modified polysiloxane          |         |                               |
|                                   | Kind of particles to be treated                  | Kind    | Amount added (part by weight) |
| Example 31                        | Core particles 1                                 | BYK-080 | 1.0                           |
| Example 32                        | Core particles 2                                 | BYK-080 | 0.5                           |
| Example 33                        | Core particles 3                                 | BYK-310 | 2.0                           |
| Example 34                        | Core particles 4                                 | BYK-322 | 5.0                           |
| Example 35                        | Core particles 5                                 | BYK-080 | 2.0                           |
| Example 36                        | Core particles 6                                 | BYK-080 | 3.0                           |
| Example 37                        | Core particles 7                                 | BYK-310 | 1.5                           |

TABLE 10-continued

|                        |                  |         |       |
|------------------------|------------------|---------|-------|
| Example 38             | Core particles 8 | BYK-322 | 7.0   |
| Comparative Example 18 | Core particles 1 | BYK-080 | 1.0   |
| Comparative Example 19 | Core particles 1 | BYK-080 | 0.5   |
| Comparative Example 20 | Core particles 1 | BYK-080 | 0.005 |

TABLE 10-continued

|                        |    |    |      |
|------------------------|----|----|------|
| Comparative Example 19 | 60 | 30 | 0.01 |
| Comparative Example 20 | 60 | 30 | 4.75 |

TABLE 11

| Production of black magnetic composite particles<br>Coating step with modified polysiloxane                      |                       |                                          |                                           | Production of black magnetic composite particles<br>Coating step with terminal-modified polysiloxane             |                                 |                               |                                           |
|------------------------------------------------------------------------------------------------------------------|-----------------------|------------------------------------------|-------------------------------------------|------------------------------------------------------------------------------------------------------------------|---------------------------------|-------------------------------|-------------------------------------------|
| Examples and                                                                                                     | Edge runner treatment |                                          | Coating amount (calculated as Si) (wt. %) | Examples and Comparative Examples                                                                                | Kind of particles to be treated | Kind                          | Amount added (part by weight)             |
|                                                                                                                  | Linear load (Kg/cm)   | Time (min)                               |                                           |                                                                                                                  |                                 |                               |                                           |
| Example 31                                                                                                       | 60                    | 60                                       | 0.18                                      | Example 39                                                                                                       | Core particles 1                | TSF4770                       | 2.0                                       |
| Example 32                                                                                                       | 30                    | 60                                       | 0.08                                      | Example 40                                                                                                       | Core particles 2                | TSF4770                       | 1.0                                       |
| Example 33                                                                                                       | 60                    | 45                                       | 0.36                                      | Example 41                                                                                                       | Core particles 3                | TSF4751                       | 0.5                                       |
| Example 34                                                                                                       | 30                    | 30                                       | 0.87                                      | Example 42                                                                                                       | Core particles 4                | TSF4751                       | 3.0                                       |
| Example 35                                                                                                       | 45                    | 30                                       | 0.36                                      | Example 43                                                                                                       | Core particles 5                | TSF4770                       | 1.0                                       |
| Example 36                                                                                                       | 45                    | 45                                       | 0.49                                      | Example 44                                                                                                       | Core particles 6                | TSF4770                       | 3.0                                       |
| Example 37                                                                                                       | 60                    | 30                                       | 0.25                                      | Example 45                                                                                                       | Core particles 7                | TSF4751                       | 0.5                                       |
| Example 38                                                                                                       | 30                    | 45                                       | 1.20                                      | Example 46                                                                                                       | Core particles 8                | TSF4751                       | 1.7                                       |
| Comparative Example 18                                                                                           | 60                    | 30                                       | 0.16                                      | Comparative Example 21                                                                                           | Core particles 1                | TSF4770                       | 1.0                                       |
| Comparative Example 19                                                                                           | 60                    | 30                                       | 0.08                                      | Comparative Example 22                                                                                           | Core particles 1                | TSF4770                       | 1.0                                       |
| Comparative Example 20                                                                                           | 60                    | 30                                       | $8.0 \times 10^{-4}$                      | Comparative Example 23                                                                                           | Core particles 1                | TSF4770                       | 0.005                                     |
| Production of black magnetic composite particles<br>Adhering step of carbon black<br>Carbon black fine particles |                       |                                          |                                           | Production of black magnetic composite particles<br>Coating step with terminal-modified polysiloxane             |                                 |                               |                                           |
| Examples and                                                                                                     | Kind                  | Amount added (part by weight)            |                                           | Examples and                                                                                                     | Edge runner treatment           |                               | Coating amount (calculated as Si) (wt. %) |
| Comparative Examples                                                                                             | Kind                  | Amount added (part by weight)            |                                           | Comparative Examples                                                                                             | Linear load (Kg/cm)             | Time (min)                    | Si) (wt. %)                               |
| Example 31                                                                                                       | A                     | 8.0                                      |                                           | Example 39                                                                                                       | 60                              | 30                            | 0.46                                      |
| Example 32                                                                                                       | A                     | 6.0                                      |                                           | Example 40                                                                                                       | 30                              | 40                            | 0.21                                      |
| Example 33                                                                                                       | B                     | 6.5                                      |                                           | Example 41                                                                                                       | 60                              | 30                            | 0.12                                      |
| Example 34                                                                                                       | C                     | 11.5                                     |                                           | Example 42                                                                                                       | 30                              | 45                            | 0.71                                      |
| Example 35                                                                                                       | A                     | 7.5                                      |                                           | Example 43                                                                                                       | 45                              | 20                            | 0.21                                      |
| Example 36                                                                                                       | A                     | 12.5                                     |                                           | Example 44                                                                                                       | 60                              | 30                            | 0.69                                      |
| Example 37                                                                                                       | B                     | 18.0                                     |                                           | Example 45                                                                                                       | 45                              | 20                            | 0.14                                      |
| Example 38                                                                                                       | C                     | 15.0                                     |                                           | Example 46                                                                                                       | 30                              | 30                            | 0.37                                      |
| Comparative Example 18                                                                                           | —                     | —                                        |                                           | Comparative Example 21                                                                                           | 60                              | 30                            | 0.26                                      |
| Comparative Example 19                                                                                           | A                     | 0.01                                     |                                           | Comparative Example 22                                                                                           | 60                              | 30                            | 0.25                                      |
| Comparative Example 20                                                                                           | B                     | 5.0                                      |                                           | Comparative Example 23                                                                                           | 60                              | 30                            | $1.2 \times 10^{-3}$                      |
| Production of black magnetic composite particles<br>Adhering step of carbon black                                |                       |                                          |                                           | Production of black magnetic composite particles<br>Adhering step of carbon black<br>Carbon black fine particles |                                 |                               |                                           |
| Examples and                                                                                                     | Edge runner treatment | Amount adhered (calculated as C) (wt. %) |                                           | Examples and                                                                                                     | Edge runner treatment           |                               | Coating amount (calculated as Si) (wt. %) |
| Comparative Examples                                                                                             | Linear load (Kg/cm)   | Time (min)                               | as C) (wt. %)                             | Comparative Examples                                                                                             | Linear load (Kg/cm)             | Time (min)                    | Si) (wt. %)                               |
| Example 31                                                                                                       | 60                    | 30                                       | 7.43                                      | Example 39                                                                                                       | 60                              | 30                            | 0.46                                      |
| Example 32                                                                                                       | 30                    | 25                                       | 5.68                                      | Example 40                                                                                                       | 30                              | 40                            | 0.21                                      |
| Example 33                                                                                                       | 30                    | 30                                       | 6.10                                      | Example 41                                                                                                       | 60                              | 30                            | 0.12                                      |
| Example 34                                                                                                       | 60                    | 20                                       | 10.24                                     | Example 42                                                                                                       | 30                              | 45                            | 0.71                                      |
| Example 35                                                                                                       | 45                    | 45                                       | 6.98                                      | Example 43                                                                                                       | 45                              | 20                            | 0.21                                      |
| Example 36                                                                                                       | 60                    | 30                                       | 11.10                                     | Example 44                                                                                                       | 60                              | 30                            | 0.69                                      |
| Example 37                                                                                                       | 30                    | 25                                       | 15.16                                     | Example 45                                                                                                       | 45                              | 20                            | 0.14                                      |
| Example 38                                                                                                       | 45                    | 40                                       | 13.10                                     | Example 46                                                                                                       | 30                              | 30                            | 0.37                                      |
| Comparative Example 18                                                                                           | —                     | —                                        |                                           | Comparative Example 21                                                                                           | 60                              | 30                            | 0.26                                      |
| Production of black magnetic composite particles<br>Adhering step of carbon black<br>Carbon black fine particles |                       |                                          |                                           | Comparative Example 22                                                                                           | 60                              | 30                            | 0.25                                      |
| Examples and                                                                                                     | Kind                  | Amount added (part by weight)            |                                           | Comparative Examples                                                                                             | Kind                            | Amount added (part by weight) |                                           |
| Comparative Examples                                                                                             | Kind                  | Amount added (part by weight)            |                                           | Example 39                                                                                                       | A                               | 10.0                          |                                           |
| Comparative Example 40                                                                                           | A                     | 6.0                                      |                                           | Example 40                                                                                                       | A                               | 6.0                           |                                           |

TABLE 11-continued

|             |   |      |    |
|-------------|---|------|----|
| Example 41  | B | 8.0  |    |
| Example 42  | C | 10.0 |    |
| Example 43  | A | 7.5  | 5  |
| Example 44  | A | 12.0 |    |
| Example 45  | B | 19.0 |    |
| Example 46  | C | 13.0 |    |
| Comparative | — | —    |    |
| Example 21  |   |      |    |
| Comparative | A | 0.01 | 10 |
| Example 22  |   |      |    |
| Comparative | B | 5.0  |    |
| Example 23  |   |      |    |

  

| Production of black magnetic composite particles |                               |                             |               |
|--------------------------------------------------|-------------------------------|-----------------------------|---------------|
| Examples and                                     | Adhering step of carbon black |                             |               |
|                                                  | Edge runner treatment         | Amount adhered (calculated) |               |
| Comparative Examples                             | Linear load (Kg/cm)           | Time (min)                  | as C) (wt. %) |
| Example 39                                       | 60                            | 30                          | 9.13          |
| Example 40                                       | 30                            | 45                          | 5.57          |
| Example 41                                       | 45                            | 60                          | 7.42          |
| Example 42                                       | 60                            | 45                          | 9.10          |
| Example 43                                       | 30                            | 30                          | 6.98          |
| Example 44                                       | 45                            | 25                          | 10.70         |
| Example 45                                       | 60                            | 45                          | 15.15         |
| Example 46                                       | 30                            | 30                          | 11.43         |
| Comparative                                      | —                             | —                           | —             |
| Example 21                                       |                               |                             |               |
| Comparative                                      | 60                            | 30                          | 0.01          |
| Example 22                                       |                               |                             |               |
| Comparative                                      | 60                            | 30                          | 4.73          |
| Example 23                                       |                               |                             |               |

TABLE 12-continued

| Properties of black magnetic composite particles |                    |                          |                                        |                                     |
|--------------------------------------------------|--------------------|--------------------------|----------------------------------------|-------------------------------------|
| Examples and Comparative Examples                | Fluidity index (—) | Blackness (L* value) (—) | Carbon black desorption percentage (%) | Thickness of carbon black Coat (μm) |
| Example 23                                       | 51                 | 17.0                     | 7.2                                    | 0.0024                              |
| Example 24                                       | 48                 | 16.5                     | 8.6                                    | 0.0021                              |
| Example 25                                       | 46                 | 17.2                     | 8.8                                    | 0.0022                              |
| Example 26                                       | 53                 | 17.4                     | 6.2                                    | 0.0024                              |
| Example 27                                       | 50                 | 15.3                     | 4.6                                    | 0.0022                              |
| Example 28                                       | 48                 | 16.0                     | 3.6                                    | 0.0025                              |
| Example 29                                       | 49                 | 17.6                     | 1.8                                    | 0.0026                              |
| Example 30                                       | 51                 | 17.6                     | 3.2                                    | 0.0024                              |
| Comparative                                      | 39                 | 20.6                     | 60.5                                   | —                                   |
| Example 15                                       |                    |                          |                                        |                                     |
| Comparative                                      | 39                 | 21.0                     | 28.3                                   | —                                   |
| Example 16                                       |                    |                          |                                        |                                     |
| Comparative                                      | 40                 | 20.8                     | 43.8                                   | —                                   |
| Example 17                                       |                    |                          |                                        |                                     |

TABLE 12

| Properties of black magnetic composite particles |                            |                  |                                    |                                               |
|--------------------------------------------------|----------------------------|------------------|------------------------------------|-----------------------------------------------|
| Examples and Comparative Examples                | Average particle size (μm) | Aspect ratio (—) | Geometrical standard deviation (—) | BET specific surface area (m <sup>2</sup> /g) |
| Example 23                                       | 0.28                       | —                | 1.52                               | 6.1                                           |
| Example 24                                       | 0.24                       | —                | 1.34                               | 12.8                                          |
| Example 25                                       | 0.41                       | 8.1:1            | 1.51                               | 24.6                                          |
| Example 26                                       | 0.23                       | —                | 1.42                               | 14.6                                          |
| Example 27                                       | 0.29                       | —                | 1.50                               | 14.3                                          |
| Example 28                                       | 0.23                       | —                | 1.34                               | 15.1                                          |
| Example 29                                       | 0.40                       | 8.1:1            | 1.50                               | 24.8                                          |
| Example 30                                       | 0.23                       | —                | 1.42                               | 12.8                                          |
| Comparative                                      | 0.29                       | —                | 1.53                               | 11.5                                          |
| Example 15                                       |                            |                  |                                    |                                               |
| Comparative                                      | 0.28                       | —                | 1.53                               | 7.1                                           |
| Example 16                                       |                            |                  |                                    |                                               |
| Comparative                                      | 0.28                       | —                | 1.53                               | 15.6                                          |
| Example 17                                       |                            |                  |                                    |                                               |

  

| Properties of black magnetic composite particles |                     |                                           |                                         |
|--------------------------------------------------|---------------------|-------------------------------------------|-----------------------------------------|
| Magnetic properties                              |                     |                                           |                                         |
| Examples and Comparative Examples                | Coercive force (Oe) | Saturation magnetization (10 kOe) (emu/g) | Residual magnetization (10 kOe) (emu/g) |
| Example 23                                       | 108                 | 80.8                                      | 11.0                                    |
| Example 24                                       | 64                  | 71.6                                      | 6.6                                     |
| Example 25                                       | 338                 | 75.2                                      | 25.8                                    |
| Example 26                                       | 56                  | 64.1                                      | 6.3                                     |

TABLE 13

| Properties of black magnetic composite particles |                            |                  |                                    |                                               |
|--------------------------------------------------|----------------------------|------------------|------------------------------------|-----------------------------------------------|
| Examples and Comparative Examples                | Average particle size (μm) | Aspect ratio (—) | Geometrical standard deviation (—) | BET specific surface area (m <sup>2</sup> /g) |
| Example 31                                       | 0.28                       | —                | 1.52                               | 6.8                                           |
| Example 32                                       | 0.23                       | —                | 1.34                               | 11.9                                          |
| Example 33                                       | 0.40                       | 8.1:1            | 1.52                               | 24.9                                          |
| Example 34                                       | 0.23                       | —                | 1.42                               | 13.8                                          |
| Example 35                                       | 0.29                       | —                | 1.51                               | 15.1                                          |
| Example 36                                       | 0.23                       | —                | 1.34                               | 14.6                                          |
| Example 37                                       | 0.41                       | 8.1:1            | 1.50                               | 25.6                                          |
| Example 38                                       | 0.23                       | —                | 1.42                               | 11.8                                          |
| Comparative                                      | 0.28                       | —                | 1.53                               | 11.3                                          |
| Example 18                                       |                            |                  |                                    |                                               |
| Comparative                                      | 0.28                       | —                | 1.52                               | 10.6                                          |
| Example 19                                       |                            |                  |                                    |                                               |
| Comparative                                      | 0.28                       | —                | 1.53                               | 16.3                                          |
| Example 20                                       |                            |                  |                                    |                                               |

  

| Properties of black magnetic composite particles |                     |                                           |                                         |  |
|--------------------------------------------------|---------------------|-------------------------------------------|-----------------------------------------|--|
| Magnetic properties                              |                     |                                           |                                         |  |
| Examples and Comparative Examples                | Coercive force (Oe) | Saturation magnetization (10 kOe) (emu/g) | Residual magnetization (10 kOe) (emu/g) |  |
| Example 31                                       | 108                 | 80.6                                      | 10.8                                    |  |
| Example 32                                       | 63                  | 71.8                                      | 7.1                                     |  |
| Example 33                                       | 336                 | 75.3                                      | 25.6                                    |  |
| Example 34                                       | 57                  | 64.6                                      | 6.1                                     |  |
| Example 35                                       | 106                 | 73.2                                      | 10.0                                    |  |
| Example 36                                       | 63                  | 75.2                                      | 6.1                                     |  |

TABLE 13-continued

|                                                  |                    |                          |                                        |                                     |
|--------------------------------------------------|--------------------|--------------------------|----------------------------------------|-------------------------------------|
| Example 37                                       | 336                | 77.8                     | 26.3                                   |                                     |
| Example 38                                       | 56                 | 65.3                     | 6.5                                    |                                     |
| Comparative Example 18                           | 102                | 78.3                     | 10.0                                   | 5                                   |
| Comparative Example 19                           | 100                | 83.2                     | 10.8                                   |                                     |
| Comparative Example 20                           | 102                | 81.6                     | 10.1                                   |                                     |
| Properties of black magnetic composite particles |                    |                          |                                        |                                     |
| Examples and Comparative Examples                | Fluidity index (→) | Blackness (L* value) (→) | Carbon black desorption percentage (%) | Thickness of carbon black Coat (μm) |
| Example 31                                       | 52                 | 17.1                     | 8.3                                    | 0.0023                              |
| Example 32                                       | 52                 | 16.8                     | 9.1                                    | 0.0022                              |
| Example 33                                       | 53                 | 17.5                     | 6.3                                    | 0.0023                              |
| Example 34                                       | 46                 | 17.0                     | 5.9                                    | 0.0024                              |
| Example 35                                       | 48                 | 17.3                     | 4.8                                    | 0.0023                              |
| Example 36                                       | 51                 | 16.1                     | 3.9                                    | 0.0024                              |
| Example 37                                       | 50                 | 16.0                     | 3.8                                    | 0.0025                              |
| Example 38                                       | 53                 | 17.3                     | 2.8                                    | 0.0025                              |
| Comparative Example 18                           | 38                 | 21.0                     | 61.3                                   | —                                   |
| Comparative Example 19                           | 37                 | 20.6                     | 27.3                                   | —                                   |
| Comparative Example 20                           | 38                 | 20.5                     | 45.9                                   | —                                   |

TABLE 14-continued

|                                                  |                    |                          |                                        |
|--------------------------------------------------|--------------------|--------------------------|----------------------------------------|
| Comparative Example 22                           | 104                | 84.1                     | 10.0                                   |
| Comparative Example 23                           | 103                | 83.1                     | 10.1                                   |
| Properties of black magnetic composite particles |                    |                          |                                        |
| 10 Examples and Comparative Examples             | Fluidity index (→) | Blackness (L* value) (→) | Carbon black desorption percentage (%) |
| 15 Example 39                                    | 52                 | 16.0                     | 7.1                                    |
| Example 40                                       | 51                 | 16.3                     | 6.5                                    |
| Example 41                                       | 53                 | 17.2                     | 5.9                                    |
| Example 42                                       | 52                 | 17.6                     | 5.3                                    |
| Example 43                                       | 54                 | 16.0                     | 4.3                                    |
| Example 44                                       | 54                 | 16.0                     | 3.4                                    |
| Example 45                                       | 52                 | 17.4                     | 3.8                                    |
| Example 46                                       | 53                 | 17.4                     | 4.3                                    |
| Comparative Example 21                           | 37                 | 20.8                     | 69.2                                   |
| Comparative Example 22                           | 37                 | 21.0                     | 31.6                                   |
| Comparative Example 23                           | 38                 | 20.6                     | 50.8                                   |

TABLE 14

|                                                  |                                                  |                                           |                                         |                                               |
|--------------------------------------------------|--------------------------------------------------|-------------------------------------------|-----------------------------------------|-----------------------------------------------|
| Examples and Comparative Examples                | Properties of black magnetic composite particles |                                           |                                         |                                               |
|                                                  | Average particle size (μm)                       | Aspect ratio (→)                          | Geometrical standard deviation (→)      | BET specific surface area (m <sup>2</sup> /g) |
| Example 39                                       | 0.28                                             | —                                         | 1.52                                    | 5.9                                           |
| Example 40                                       | 0.23                                             | —                                         | 1.34                                    | 12.6                                          |
| Example 41                                       | 0.41                                             | 8.0:1                                     | 1.52                                    | 25.6                                          |
| Example 42                                       | 0.23                                             | —                                         | 1.43                                    | 13.9                                          |
| Example 43                                       | 0.29                                             | —                                         | 1.50                                    | 14.8                                          |
| Example 44                                       | 0.23                                             | —                                         | 1.34                                    | 16.3                                          |
| Example 45                                       | 0.40                                             | 8.1:1                                     | 1.50                                    | 21.8                                          |
| Example 46                                       | 0.23                                             | —                                         | 1.43                                    | 13.6                                          |
| Comparative Example 21                           | 0.29                                             | —                                         | 1.52                                    | 10.3                                          |
| Comparative Example 22                           | 0.29                                             | —                                         | 1.51                                    | 10.6                                          |
| Comparative Example 23                           | 0.29                                             | —                                         | 1.52                                    | 10.1                                          |
| Properties of black magnetic composite particles |                                                  |                                           |                                         |                                               |
| Magnetic properties                              |                                                  |                                           |                                         |                                               |
| Examples and Comparative Examples                | Coercive force (Oe)                              | Saturation magnetization (10 kOe) (emu/g) | Residual magnetization (10 kOe) (emu/g) |                                               |
| Example 39                                       | 107                                              | 81.4                                      | 11.6                                    |                                               |
| Example 40                                       | 66                                               | 72.1                                      | 6.3                                     |                                               |
| Example 41                                       | 341                                              | 74.1                                      | 25.4                                    |                                               |
| Example 42                                       | 59                                               | 63.6                                      | 6.0                                     |                                               |
| Example 43                                       | 107                                              | 73.1                                      | 10.1                                    |                                               |
| Example 44                                       | 66                                               | 73.8                                      | 6.6                                     |                                               |
| Example 45                                       | 340                                              | 78.1                                      | 26.8                                    |                                               |
| Example 46                                       | 56                                               | 66.6                                      | 6.8                                     |                                               |
| Comparative Example 21                           | 104                                              | 83.1                                      | 10.0                                    |                                               |

TABLE 15

|                                      |                                    |                                 |                               |                                 |
|--------------------------------------|------------------------------------|---------------------------------|-------------------------------|---------------------------------|
| 30                                   | Production of black magnetic toner |                                 |                               |                                 |
|                                      | Black magnetic composite particles |                                 |                               |                                 |
| 35 Examples and Comparative Examples | Kind                               | Amount blended (part by weight) | Kind                          | Amount blended (part by weight) |
| 40 Example 47                        | Example 23                         | 45                              | Styrene-acryl copolymer resin | 55                              |
| Example 48                           | Example 24                         | 45                              | Styrene-acryl copolymer resin | 55                              |
| 45 Example 49                        | Example 25                         | 40                              | Styrene-acryl copolymer resin | 60                              |
| Example 50                           | Example 26                         | 50                              | Styrene-acryl copolymer resin | 50                              |
| Example 51                           | Example 27                         | 45                              | Styrene-acryl copolymer resin | 55                              |
| Example 52                           | Example 28                         | 40                              | Styrene-acryl copolymer resin | 60                              |
| Example 53                           | Example 29                         | 50                              | Styrene-acryl copolymer resin | 50                              |
| Example 54                           | Example 30                         | 50                              | Styrene-acryl copolymer resin | 50                              |
| Comparative Example 24               | Comparative Example 15             | 45                              | Styrene-acryl copolymer resin | 55                              |
| Comparative Example 25               | Comparative Example 16             | 45                              | Styrene-acryl copolymer resin | 55                              |
| Comparative Example 26               | Comparative Example 17             | 45                              | Styrene-acryl copolymer resin | 55                              |

TABLE 15-continued

| Properties of black magnetic toner |                                         |                    |                    |                                                 |
|------------------------------------|-----------------------------------------|--------------------|--------------------|-------------------------------------------------|
| Examples and Comparative Examples  | Average particle size ( $\mu\text{m}$ ) | Dispersibility (-) | Fluidity index (-) | Volume resistivity ( $\Omega \cdot \text{cm}$ ) |
| Example 47                         | 9.9                                     | 5                  | 75                 | $8.9 \times 10^{13}$                            |
| Example 48                         | 10.0                                    | 5                  | 81                 | $1.8 \times 10^{14}$                            |
| Example 49                         | 10.6                                    | 4                  | 75                 | $7.6 \times 10^{13}$                            |
| Example 50                         | 10.5                                    | 5                  | 78                 | $7.1 \times 10^{13}$                            |
| Example 51                         | 9.6                                     | 5                  | 79                 | $5.9 \times 10^{13}$                            |
| Example 52                         | 9.9                                     | 5                  | 83                 | $3.1 \times 10^{14}$                            |
| Example 53                         | 10.0                                    | 5                  | 76                 | $1.9 \times 10^{14}$                            |
| Example 54                         | 10.8                                    | 5                  | 83                 | $1.5 \times 10^{14}$                            |
| Comparative Example 24             | 10.6                                    | 2                  | 56                 | $1.8 \times 10^{12}$                            |
| Comparative Example 25             | 10.5                                    | 2                  | 58                 | $2.1 \times 10^{12}$                            |
| Comparative Example 26             | 10.4                                    | 2                  | 56                 | $2.1 \times 10^{12}$                            |

  

| Properties of black magnetic toner |                     |                                           |                                          |
|------------------------------------|---------------------|-------------------------------------------|------------------------------------------|
| Magnetic properties                |                     |                                           |                                          |
| Examples and Comparative Examples  | Coercive force (Oe) | Saturation magnetization (10 kOe) (emu/g) | Saturation magnetization (1 kOe) (emu/g) |
| Example 47                         | 97                  | 36.6                                      | 27.4                                     |
| Example 48                         | 60                  | 33.4                                      | 26.0                                     |
| Example 49                         | 321                 | 31.4                                      | 23.5                                     |
| Example 50                         | 57                  | 32.3                                      | 22.8                                     |
| Example 51                         | 104                 | 32.5                                      | 23.5                                     |
| Example 52                         | 67                  | 29.8                                      | 22.6                                     |
| Example 53                         | 328                 | 33.6                                      | 23.6                                     |
| Example 54                         | 52                  | 31.7                                      | 24.1                                     |
| Comparative Example 24             | 101                 | 37.2                                      | 27.2                                     |
| Comparative Example 25             | 102                 | 38.0                                      | 29.3                                     |
| Comparative Example 26             | 102                 | 36.5                                      | 28.5                                     |

  

| Properties of black magnetic toner |                     |                                         |                                        |                          |
|------------------------------------|---------------------|-----------------------------------------|----------------------------------------|--------------------------|
| Examples and Comparative Examples  | Magnetic properties | Residual magnetization (10 kOe) (emu/g) | Residual magnetization (1 kOe) (emu/g) | Blackness (L* value) (-) |
| Example 47                         | 5.8                 | 4.3                                     | 18.5                                   |                          |
| Example 48                         | 4.1                 | 2.9                                     | 17.9                                   |                          |
| Example 49                         | 11.1                | 8.4                                     | 19.2                                   |                          |
| Example 50                         | 4.4                 | 3.2                                     | 19.3                                   |                          |
| Example 51                         | 5.3                 | 4.0                                     | 17.6                                   |                          |
| Example 52                         | 3.7                 | 2.8                                     | 18.2                                   |                          |
| Example 53                         | 10.1                | 7.2                                     | 18.0                                   |                          |
| Example 54                         | 4.7                 | 3.1                                     | 19.1                                   |                          |
| Comparative Example 24             | 5.1                 | 4.0                                     | 22.2                                   |                          |
| Comparative Example 25             | 5.1                 | 4.0                                     | 23.6                                   |                          |
| Comparative Example 26             | 5.0                 | 4.1                                     | 23.0                                   |                          |

TABLE 16

| Production of black magnetic toner |                                    |                                 |                               |                                 |
|------------------------------------|------------------------------------|---------------------------------|-------------------------------|---------------------------------|
| Examples and Comparative Examples  | Black magnetic composite particles |                                 | Resin                         |                                 |
|                                    | Kind                               | Amount blended (part by weight) | Kind                          | Amount blended (part by weight) |
| Example 55                         | Example 31                         | 45                              | Styrene-acryl copolymer resin | 55                              |
| Example 56                         | Example 32                         | 45                              | Styrene-acryl copolymer resin | 55                              |
| Example 57                         | Example 33                         | 40                              | Styrene-acryl copolymer resin | 60                              |
| Example 58                         | Example 34                         | 50                              | Styrene-acryl copolymer resin | 50                              |
| Example 59                         | Example 35                         | 45                              | Styrene-acryl copolymer resin | 55                              |
| Example 60                         | Example 36                         | 40                              | Styrene-acryl copolymer resin | 60                              |
| Example 61                         | Example 37                         | 50                              | Styrene-acryl copolymer resin | 50                              |
| Example 62                         | Example 38                         | 50                              | Styrene-acryl copolymer resin | 50                              |
| Comparative Example 27             | Comparative Example 18             | 45                              | Styrene-acryl copolymer resin | 55                              |
| Comparative Example 28             | Comparative Example 19             | 45                              | Styrene-acryl copolymer resin | 55                              |
| Comparative Example 29             | Comparative Example 20             | 45                              | Styrene-acryl copolymer resin | 55                              |

  

| Properties of black magnetic toner |                                         |                    |                    |                                                 |
|------------------------------------|-----------------------------------------|--------------------|--------------------|-------------------------------------------------|
| Examples and Comparative Examples  | Average particle size ( $\mu\text{m}$ ) | Dispersibility (-) | Fluidity index (-) | Volume resistivity ( $\Omega \cdot \text{cm}$ ) |
| Example 55                         | 10.0                                    | 5                  | 76                 | $9.2 \times 10^{13}$                            |
| Example 56                         | 10.0                                    | 5                  | 80                 | $2.5 \times 10^{14}$                            |
| Example 57                         | 10.1                                    | 4                  | 76                 | $6.5 \times 10^{13}$                            |
| Example 58                         | 9.9                                     | 5                  | 81                 | $7.8 \times 10^{13}$                            |
| Example 59                         | 10.1                                    | 5                  | 80                 | $7.3 \times 10^{13}$                            |
| Example 60                         | 9.8                                     | 5                  | 85                 | $3.2 \times 10^{14}$                            |
| Example 61                         | 10.2                                    | 5                  | 75                 | $2.6 \times 10^{14}$                            |
| Comparative Example 27             | 10.4                                    | 2                  | 59                 | $3.1 \times 10^{12}$                            |
| Comparative Example 28             | 10.2                                    | 2                  | 60                 | $3.4 \times 10^{12}$                            |

  

| Properties of black magnetic toner |                     |                     |                                         |                                        |
|------------------------------------|---------------------|---------------------|-----------------------------------------|----------------------------------------|
| Examples and Comparative Examples  | Magnetic properties | Coercive force (Oe) | Residual magnetization (10 kOe) (emu/g) | Residual magnetization (1 kOe) (emu/g) |
| Example 55                         | 5.8                 | 4.3                 | 18.5                                    |                                        |
| Example 56                         | 4.1                 | 2.9                 | 17.9                                    |                                        |
| Example 57                         | 11.1                | 8.4                 | 19.2                                    |                                        |
| Example 58                         | 4.4                 | 3.2                 | 19.3                                    |                                        |
| Example 59                         | 5.3                 | 4.0                 | 17.6                                    |                                        |
| Example 60                         | 3.7                 | 2.8                 | 18.2                                    |                                        |
| Example 61                         | 10.1                | 7.2                 | 18.0                                    |                                        |
| Comparative Example 28             | 4.7                 | 3.1                 | 19.1                                    |                                        |
| Comparative Example 29             | 5.1                 | 4.0                 | 22.2                                    |                                        |

  

| Properties of black magnetic toner |                     |                     |                                         |                                        |
|------------------------------------|---------------------|---------------------|-----------------------------------------|----------------------------------------|
| Examples and Comparative Examples  | Magnetic properties | Coercive force (Oe) | Residual magnetization (10 kOe) (emu/g) | Residual magnetization (1 kOe) (emu/g) |
| Example 55                         | 5.8                 | 4.3                 | 18.5                                    |                                        |
| Example 56                         | 4.1                 | 2.9                 | 17.9                                    |                                        |
| Example 57                         | 11.1                | 8.4                 | 19.2                                    |                                        |
| Example 58                         | 4.4                 | 3.2                 | 19.3                                    |                                        |
| Example 59                         | 5.3                 | 4.0                 | 17.6                                    |                                        |
| Example 60                         | 3.7                 | 2.8                 | 18.2                                    |                                        |
| Example 61                         | 10.1                | 7.2                 | 18.0                                    |                                        |
| Comparative Example 28             | 4.7                 | 3.1                 | 19.1                                    |                                        |
| Comparative Example 29             | 5.1                 | 4.0                 | 22.2                                    |                                        |

TABLE 16-continued

|                                    |          |                        |            |           |
|------------------------------------|----------|------------------------|------------|-----------|
| Example 60                         | 66       | 29.4                   | 22.1       |           |
| Example 61                         | 318      | 33.4                   | 25.6       |           |
| Example 62                         | 51       | 31.6                   | 23.4       |           |
| Comparative Example 27             | 101      | 38.2                   | 27.8       |           |
| Comparative Example 28             | 102      | 38.2                   | 29.3       |           |
| Comparative Example 29             | 100      | 36.7                   | 28.5       |           |
| Properties of black magnetic toner |          |                        |            |           |
| Examples and Comparative Examples  |          | Magnetic properties    |            |           |
|                                    |          | Residual magnetization |            |           |
| Comparative Examples               | (10 kOe) | (1 kOe)                | (L* value) | Blackness |
| (emu/g)                            | (emu/g)  | (-)                    |            |           |
| Example 55                         | 5.8      | 4.3                    | 18.4       |           |
| Example 56                         | 4.1      | 2.8                    | 17.9       |           |
| Example 57                         | 11.4     | 8.6                    | 19.3       |           |
| Example 58                         | 4.5      | 3.3                    | 18.8       |           |
| Example 59                         | 5.3      | 4.1                    | 17.2       |           |
| Example 60                         | 3.7      | 2.8                    | 17.9       |           |
| Example 61                         | 8.6      | 6.4                    | 18.3       |           |
| Example 62                         | 4.3      | 3.1                    | 18.6       |           |
| Comparative Example 27             | 5.9      | 4.6                    | 23.3       |           |
| Comparative Example 28             | 5.3      | 4.1                    | 22.8       |           |
| Comparative Example 29             | 5.0      | 3.9                    | 22.2       |           |

TABLE 17

|                                    |                        |                                 |                               |                                 |    |  |  |
|------------------------------------|------------------------|---------------------------------|-------------------------------|---------------------------------|----|--|--|
|                                    |                        |                                 |                               |                                 |    |  |  |
| Production of black magnetic toner |                        |                                 |                               |                                 |    |  |  |
| Black magnetic composite particles |                        |                                 |                               |                                 |    |  |  |
| Resin                              |                        |                                 |                               |                                 |    |  |  |
| Examples and Comparative Examples  | Kind                   | Amount blended (part by weight) | Kind                          | Amount blended (part by weight) |    |  |  |
| Example 63                         | Example 39             | 45                              | Styrene-acryl copolymer resin | 55                              |    |  |  |
| Example 64                         | Example 40             | 45                              | Styrene-acryl copolymer resin | 55                              | 45 |  |  |
| Example 65                         | Example 41             | 40                              | Styrene-acryl copolymer resin | 60                              |    |  |  |
| Example 66                         | Example 42             | 50                              | Styrene-acryl copolymer resin | 50                              | 50 |  |  |
| Example 67                         | Example 43             | 45                              | Styrene-acryl copolymer resin | 55                              |    |  |  |
| Example 68                         | Example 44             | 40                              | Styrene-acryl copolymer resin | 60                              | 55 |  |  |
| Example 69                         | Example 45             | 50                              | Styrene-acryl copolymer resin | 50                              |    |  |  |
| Example 70                         | Example 46             | 50                              | Styrene-acryl copolymer resin | 50                              | 60 |  |  |
| Comparative Example 30             | Comparative Example 21 | 45                              | Styrene-acryl copolymer resin | 55                              |    |  |  |
| Comparative Example 31             | Comparative Example 22 | 45                              | Styrene-acryl copolymer resin | 55                              | 65 |  |  |

TABLE 17-continued

|    |                                    |                                         |                                    |                               |                                                 |
|----|------------------------------------|-----------------------------------------|------------------------------------|-------------------------------|-------------------------------------------------|
| 5  | Comparative Example 32             | Comparative Example 23                  | 45                                 | Styrene-acryl copolymer resin | 55                                              |
|    |                                    |                                         | Properties of black magnetic toner |                               |                                                 |
| 10 | Examples and Comparative Examples  | Average particle size ( $\mu\text{m}$ ) | Dispersibility (-)                 | Fluidity index (-)            | Volume resistivity ( $\Omega \cdot \text{cm}$ ) |
| 15 | Example 63                         | 10.1                                    | 5                                  | 75                            | $8.6 \times 10^{13}$                            |
|    | Example 64                         | 9.8                                     | 5                                  | 78                            | $2.1 \times 10^{14}$                            |
|    | Example 65                         | 10.2                                    | 4                                  | 72                            | $6.5 \times 10^{13}$                            |
|    | Example 66                         | 9.9                                     | 5                                  | 80                            | $7.3 \times 10^{13}$                            |
|    | Example 67                         | 10.3                                    | 5                                  | 80                            | $7.1 \times 10^{13}$                            |
|    | Example 68                         | 10.0                                    | 5                                  | 82                            | $3.2 \times 10^{14}$                            |
|    | Example 69                         | 9.6                                     | 5                                  | 79                            | $1.6 \times 10^{14}$                            |
|    | Example 70                         | 10.0                                    | 5                                  | 83                            | $2.1 \times 10^{14}$                            |
|    | Comparative Example 30             | 9.8                                     | 2                                  | 59                            | $1.2 \times 10^{12}$                            |
|    | Comparative Example 31             | 9.9                                     | 2                                  | 57                            | $1.4 \times 10^{12}$                            |
|    | Comparative Example 32             | 10.0                                    | 2                                  | 57                            | $3.2 \times 10^{12}$                            |
| 20 | Properties of black magnetic toner |                                         |                                    |                               |                                                 |
| 25 | Examples and Comparative Examples  | Coercive force (Oe)                     | (10 kOe) (emu/g)                   | (1 kOe) (emu/g)               |                                                 |
| 30 | Comparative Examples               |                                         |                                    |                               |                                                 |
| 35 | Example 63                         | 98                                      | 36.9                               | 27.3                          |                                                 |
|    | Example 64                         | 62                                      | 33.8                               | 26.2                          |                                                 |
|    | Example 65                         | 308                                     | 34.9                               | 23.1                          |                                                 |
|    | Example 66                         | 58                                      | 32.6                               | 22.6                          |                                                 |
|    | Example 67                         | 101                                     | 32.6                               | 23.1                          |                                                 |
|    | Example 68                         | 64                                      | 32.6                               | 22.6                          |                                                 |
|    | Example 69                         | 313                                     | 33.2                               | 24.2                          |                                                 |
|    | Example 70                         | 56                                      | 32.1                               | 23.1                          |                                                 |
|    | Comparative Example 30             | 102                                     | 38.6                               | 27.3                          |                                                 |
|    | Comparative Example 31             | 103                                     | 37.9                               | 25.6                          |                                                 |
| 40 | Comparative Examples               |                                         |                                    |                               |                                                 |
| 45 | Properties of black magnetic toner |                                         |                                    |                               |                                                 |
| 50 | Examples and Comparative Examples  | Magnetic properties                     | Residual magnetization             | Blackness                     |                                                 |
| 55 | Example 63                         | (10 kOe) (emu/g)                        | (1 kOe) (emu/g)                    | (L* value) (-)                |                                                 |
| 60 | Example 64                         | 5.6                                     | 4.2                                | 18.6                          |                                                 |
|    | Example 65                         | 3.6                                     | 2.8                                | 17.8                          |                                                 |
|    | Example 66                         | 12.1                                    | 8.4                                | 19.0                          |                                                 |
|    | Example 67                         | 3.6                                     | 3.1                                | 18.6                          |                                                 |
|    | Example 68                         | 5.1                                     | 3.9                                | 17.4                          |                                                 |
|    | Example 69                         | 3.8                                     | 2.5                                | 18.0                          |                                                 |
|    | Example 70                         | 10.6                                    | 5.2                                | 18.3                          |                                                 |
|    | Comparative Example 30             | 4.3                                     | 3.4                                | 18.9                          |                                                 |
|    | Comparative Example 31             | 5.8                                     | 4.3                                | 23.2                          |                                                 |
|    | Comparative Example 32             | 5.3                                     | 4.2                                | 23.5                          |                                                 |
|    | Comparative Example 33             | 5.0                                     | 4.0                                | 23.1                          |                                                 |
| 65 |                                    |                                         |                                    |                               |                                                 |

TABLE 18

| Production of black magnetic composite particles |                                 |                                       |                               |
|--------------------------------------------------|---------------------------------|---------------------------------------|-------------------------------|
| Coating step with fluoroalkylsilane compound     |                                 |                                       |                               |
| Fluoroalkylsilane compound                       |                                 |                                       |                               |
| Examples and Comparative Examples                | Kind of particles to be treated | Kind                                  | Amount added (part by weight) |
| Example 71                                       | Core particles 1                | Tridecafluoroctyl trimethoxysilane    | 2.0                           |
| Example 72                                       | Core particles 2                | Heptadecafluorodecyl trimethoxysilane | 4.0                           |
| Example 73                                       | Core particles 3                | Trifluoropropyl trimethoxysilane      | 3.0                           |
| Example 74                                       | Core particles 4                | Tridecafluoroctyl trimethoxysilane    | 1.0                           |
| Example 75                                       | Core particles 5                | Tridecafluoroctyl trimethoxysilane    | 6.0                           |
| Example 76                                       | Core particles 6                | Heptadecafluorodecyl trimethoxysilane | 4.0                           |
| Example 77                                       | Core particles 7                | Trifluoropropyl trimethoxysilane      | 0.5                           |
| Example 78                                       | Core particles 8                | Tridecafluoroctyl trimethoxysilane    | 1.5                           |
| Comparative Example 33                           | Core particles 1                | Tridecafluoroctyl trimethoxysilane    | 2.0                           |
| Comparative Example 34                           | Core particles 1                | Tridecafluoroctyl trimethoxysilane    | 3.0                           |
| Comparative Example 35                           | Core particles 1                | Tridecafluoroctyl trimethoxysilane    | 0.005                         |
| Production of black magnetic composite particles |                                 |                                       |                               |
| Coating step with fluoroalkylsilane compound     |                                 |                                       |                               |
| Examples and                                     | Edge runner treatment           |                                       | Coating amount (calculated)   |
| Comparative Examples                             | Linear load (Kg/cm)             | Time (min)                            | as Si) (wt. %)                |
| Example 71                                       | 60                              | 30                                    | 0.13                          |
| Example 72                                       | 45                              | 25                                    | 0.20                          |
| Example 73                                       | 30                              | 40                                    | 0.47                          |
| Example 74                                       | 75                              | 45                                    | 0.07                          |
| Example 75                                       | 60                              | 30                                    | 0.39                          |
| Example 76                                       | 60                              | 20                                    | 0.21                          |
| Example 77                                       | 30                              | 45                                    | 0.08                          |
| Example 78                                       | 30                              | 60                                    | 0.10                          |
| Comparative Example 33                           | 60                              | 30                                    | 0.13                          |
| Comparative Example 34                           | 60                              | 30                                    | 0.21                          |
| Comparative Example 35                           | 60                              | 30                                    | $3.0 \times 10^{-4}$          |
| Production of black magnetic composite particles |                                 |                                       |                               |
| Adhering step of carbon black                    |                                 |                                       |                               |
| Carbon black fine particles                      |                                 |                                       |                               |
| Examples and                                     | Kind                            | Amount added (part by weight)         |                               |
| Comparative Examples                             | A                               | 8.0                                   |                               |
| Example 71                                       | A                               | 6.0                                   |                               |
| Example 73                                       | B                               | 5.0                                   |                               |
| Example 74                                       | C                               | 13.0                                  |                               |
| Example 75                                       | A                               | 10.0                                  |                               |
| Example 76                                       | A                               | 10.0                                  |                               |
| Example 77                                       | B                               | 18.0                                  |                               |
| Example 78                                       | C                               | 16.0                                  |                               |
| Comparative Example 33                           | —                               | —                                     |                               |
| Comparative Example 34                           | A                               | 0.01                                  |                               |
| Comparative Example 35                           | B                               | 5.0                                   |                               |

TABLE 18-continued

| Production of black magnetic composite particles |                      |                       |                             |
|--------------------------------------------------|----------------------|-----------------------|-----------------------------|
| Adhering step of carbon black                    |                      |                       |                             |
| Examples and                                     | Comparative Examples | Edge runner treatment | Amount adhered (calculated) |
|                                                  |                      | Linear load (Kg/cm)   | as C) (wt. %)               |
| Example 71                                       | Example 71           | 60                    | 7.41                        |
| Example 72                                       | Example 72           | 30                    | 5.69                        |
| Example 73                                       | Example 73           | 60                    | 4.79                        |
| Example 74                                       | Example 74           | 30                    | 11.53                       |
| Example 75                                       | Example 75           | 60                    | 9.00                        |
| Example 76                                       | Example 76           | 30                    | 9.10                        |
| Example 77                                       | Example 77           | 60                    | 15.17                       |
| Example 78                                       | Example 78           | 30                    | 13.82                       |
| Comparative Example 33                           | —                    | —                     | —                           |
| Comparative Example 34                           | —                    | —                     | —                           |
| Comparative Example 35                           | —                    | —                     | —                           |

TABLE 19

| Properties of black magnetic composite particles |                                         |                                           |                                         |                                                     |  |
|--------------------------------------------------|-----------------------------------------|-------------------------------------------|-----------------------------------------|-----------------------------------------------------|--|
| Examples and Comparative Examples                | Average particle size ( $\mu\text{m}$ ) | Aspect ratio (—)                          | Geometrical standard deviation (—)      | BET specific surface area ( $\text{m}^2/\text{g}$ ) |  |
| Example 71                                       | 0.29                                    | —                                         | 1.53                                    | 6.3                                                 |  |
| Example 72                                       | 0.23                                    | —                                         | 1.33                                    | 12.8                                                |  |
| Example 73                                       | 0.40                                    | 8.1:1                                     | 1.52                                    | 26.8                                                |  |
| Example 74                                       | 0.23                                    | —                                         | 1.43                                    | 14.6                                                |  |
| Example 75                                       | 0.29                                    | —                                         | 1.53                                    | 15.3                                                |  |
| Example 76                                       | 0.23                                    | —                                         | 1.33                                    | 14.8                                                |  |
| Example 77                                       | 0.40                                    | 8.1:1                                     | 1.51                                    | 28.8                                                |  |
| Example 78                                       | 0.23                                    | —                                         | 1.43                                    | 13.4                                                |  |
| Comparative Example 33                           | 0.28                                    | —                                         | 1.52                                    | 10.0                                                |  |
| Comparative Example 34                           | 0.29                                    | —                                         | 1.52                                    | 9.8                                                 |  |
| Comparative Example 35                           | 0.29                                    | —                                         | 1.52                                    | 13.6                                                |  |
| Properties of black magnetic composite particles |                                         |                                           |                                         |                                                     |  |
| Magnetic properties                              |                                         |                                           |                                         |                                                     |  |
| Examples and                                     | Coercive force (Oe)                     | Saturation magnetization (10 kOe) (emu/g) | Residual magnetization (10 kOe) (emu/g) |                                                     |  |
| Comparative Examples                             |                                         |                                           |                                         |                                                     |  |
| Example 71                                       | 108                                     | 81.5                                      | 11.7                                    |                                                     |  |
| Example 72                                       | 68                                      | 72.4                                      | 6.5                                     |                                                     |  |
| Example 73                                       | 343                                     | 74.6                                      | 25.3                                    |                                                     |  |
| Example 74                                       | 58                                      | 64.3                                      | 6.1                                     |                                                     |  |
| Example 75                                       | 107                                     | 73.2                                      | 10.0                                    |                                                     |  |
| Example 76                                       | 67                                      | 73.6                                      | 6.5                                     |                                                     |  |
| Example 77                                       | 340                                     | 78.1                                      | 26.3                                    |                                                     |  |
| Example 78                                       | 57                                      | 63.2                                      | 6.5                                     |                                                     |  |
| Comparative Example 33                           | 103                                     | 83.3                                      | 9.9                                     |                                                     |  |
| Comparative Example 34                           | 103                                     | 84.1                                      | 9.8                                     |                                                     |  |
| Comparative Example 35                           | 103                                     | 83.3                                      | 10.2                                    |                                                     |  |

TABLE 19-continued

| Properties of black magnetic composite particles |                    |                      |                                        |                                     |
|--------------------------------------------------|--------------------|----------------------|----------------------------------------|-------------------------------------|
| Examples and Comparative Examples                | Fluidity index (—) | Blackness (L* value) | Carbon black desorption percentage (%) | Thickness of carbon black Coat (μm) |
| Example 71                                       | 47                 | 16.4                 | 6.1                                    | 0.0024                              |
| Example 72                                       | 48                 | 16.8                 | 7.4                                    | 0.0022                              |
| Example 73                                       | 50                 | 17.3                 | 8.2                                    | 0.0023                              |
| Example 74                                       | 46                 | 17.8                 | 5.6                                    | 0.0024                              |
| Example 75                                       | 51                 | 16.5                 | 4.3                                    | 0.0023                              |
| Example 76                                       | 52                 | 16.3                 | 4.1                                    | 0.0025                              |
| Example 77                                       | 53                 | 17.6                 | 3.8                                    | 0.0026                              |
| Example 78                                       | 52                 | 17.8                 | 4.8                                    | 0.0025                              |
| Comparative Example 33                           | 38                 | 20.6                 | 79.1                                   | —                                   |
| Comparative Example 34                           | 38                 | 20.8                 | 28.7                                   | —                                   |
| Comparative Example 35                           | 37                 | 20.3                 | 53.4                                   | —                                   |

TABLE 20

| Production of black magnetic toner |                        |                                 |                               |                                 |
|------------------------------------|------------------------|---------------------------------|-------------------------------|---------------------------------|
| Black magnetic particles           |                        |                                 | Resin                         |                                 |
| Examples and Comparative Examples  | Kind                   | Amount blended (part by weight) | Kind                          | Amount blended (part by weight) |
| Example 79                         | Example 71             | 45                              | Styrene-acryl copolymer resin | 55                              |
| Example 80                         | Example 72             | 45                              | Styrene-acryl copolymer resin | 55                              |
| Example 81                         | Example 73             | 40                              | Styrene-acryl copolymer resin | 60                              |
| Example 82                         | Example 74             | 50                              | Styrene-acryl copolymer resin | 50                              |
| Example 83                         | Example 75             | 45                              | Styrene-acryl copolymer resin | 55                              |
| Example 84                         | Example 76             | 40                              | Styrene-acryl copolymer resin | 60                              |
| Example 85                         | Example 77             | 50                              | Styrene-acryl copolymer resin | 50                              |
| Example 86                         | Example 78             | 50                              | Styrene-acryl copolymer resin | 50                              |
| Comparative Example 36             | Comparative Example 33 | 45                              | Styrene-acryl copolymer resin | 55                              |
| Comparative Example 37             | Comparative Example 34 | 45                              | Styrene-acryl copolymer resin | 55                              |
| Comparative Example 38             | Comparative Example 35 | 45                              | Styrene-acryl copolymer resin | 55                              |

TABLE 20-continued

| Properties of black magnetic toner      |                            |                                           |                    |                             |  |  |
|-----------------------------------------|----------------------------|-------------------------------------------|--------------------|-----------------------------|--|--|
| Examples and Comparative Examples       | Average particle size (μm) | Dispersibility (—)                        | Fluidity index (—) | Volume resistivity (Ω · cm) |  |  |
| Example 79                              | 10.0                       | 5                                         | 76                 | $8.1 \times 10^{13}$        |  |  |
| Example 80                              | 9.8                        | 4                                         | 81                 | $2.1 \times 10^{14}$        |  |  |
| Example 81                              | 10.1                       | 4                                         | 73                 | $6.5 \times 10^{13}$        |  |  |
| Example 82                              | 10.3                       | 5                                         | 82                 | $9.2 \times 10^{13}$        |  |  |
| Example 83                              | 10.2                       | 5                                         | 85                 | $5.4 \times 10^{13}$        |  |  |
| Example 84                              | 10.0                       | 5                                         | 86                 | $3.6 \times 10^{14}$        |  |  |
| Example 85                              | 9.9                        | 5                                         | 83                 | $2.6 \times 10^{14}$        |  |  |
| Example 86                              | 9.8                        | 5                                         | 84                 | $3.8 \times 10^{14}$        |  |  |
| Comparative Example 36                  | 10.1                       | 2                                         | 57                 | $1.3 \times 10^{12}$        |  |  |
| Comparative Example 37                  | 10.3                       | 2                                         | 56                 | $2.4 \times 10^{12}$        |  |  |
| Comparative Example 38                  | 10.1                       | 2                                         | 56                 | $6.8 \times 10^{12}$        |  |  |
| Properties of black magnetic toner      |                            |                                           |                    |                             |  |  |
| Magnetic properties                     |                            |                                           |                    |                             |  |  |
| Examples and Comparative Examples       | Coercive force (Oe)        | Saturation magnetization (10 kOe) (emu/g) |                    | (1 kOe) (emu/g)             |  |  |
| Example 79                              | 100                        | 36.9                                      |                    | 27.0                        |  |  |
| Example 80                              | 63                         | 34.8                                      |                    | 26.4                        |  |  |
| Example 81                              | 315                        | 34.3                                      |                    | 22.9                        |  |  |
| Example 82                              | 58                         | 31.6                                      |                    | 22.6                        |  |  |
| Example 83                              | 101                        | 32.1                                      |                    | 23.3                        |  |  |
| Example 84                              | 61                         | 32.8                                      |                    | 22.2                        |  |  |
| Example 85                              | 313                        | 32.6                                      |                    | 24.1                        |  |  |
| Example 86                              | 55                         | 32.1                                      |                    | 23.0                        |  |  |
| Comparative Example 36                  | 101                        | 38.4                                      |                    | 27.3                        |  |  |
| Comparative Example 37                  | 100                        | 38.0                                      |                    | 25.3                        |  |  |
| Comparative Example 38                  | 101                        | 37.1                                      |                    | 27.2                        |  |  |
| Properties of black magnetic toner      |                            |                                           |                    |                             |  |  |
| Examples and Comparative Examples       | Magnetic properties        |                                           |                    | Blackness                   |  |  |
| Residual magnetization (10 kOe) (emu/g) |                            |                                           | (L* value) (—)     |                             |  |  |
| Example 79                              | 5.7                        | 4.1                                       |                    | 18.5                        |  |  |
| Example 80                              | 3.7                        | 2.8                                       |                    | 17.6                        |  |  |
| Example 81                              | 12.3                       | 8.3                                       |                    | 18.8                        |  |  |
| Example 82                              | 3.8                        | 3.0                                       |                    | 18.6                        |  |  |
| Example 83                              | 5.6                        | 3.4                                       |                    | 17.2                        |  |  |
| Example 84                              | 3.6                        | 2.1                                       |                    | 18.3                        |  |  |
| Example 85                              | 9.8                        | 5.3                                       |                    | 17.3                        |  |  |
| Example 86                              | 3.7                        | 3.2                                       |                    | 17.3                        |  |  |
| Comparative Example 36                  | 5.4                        | 4.3                                       |                    | 23.4                        |  |  |
| Comparative Example 37                  | 5.3                        | 4.5                                       |                    | 23.2                        |  |  |
| Comparative Example 38                  | 5.0                        | 4.0                                       |                    | 22.2                        |  |  |

What is claimed is:

1. Black magnetic composite particles for a black magnetic toner, comprising:
  - maghemite particles having an average particle diameter of 0.055 to 0.95 μm;
  - a coating layer formed on the surface of said maghemite particles, comprising at least one organosilicon compound selected from the group consisting of:
    - (1) organosilane compounds obtainable from alkoxysilane compounds,
    - (2) polysiloxanes or modified polysiloxanes, and

55

(3) fluoroalkyl organosilane compounds obtainable from fluoroalkylsilane compounds; and a carbon black coat formed on said coating layer comprising said organosilicon compound, in an amount of 1 to 25 parts by weight based on 100 parts by weight of said maghemite particles.

2. Black magnetic composite particles according to claim 1, wherein said maghemite particles are particles having a coat which is formed on at least a part of the surface of said maghemite particles and which comprises at least one compound selected from the group consisting of hydroxides of aluminum, oxides of aluminum, hydroxides of silicon and oxides of silicon in an amount of 0.01 to 50% by weight, calculated as Al or SiO<sub>2</sub>, based on the total weight of the maghemite particles.

3. Black magnetic composite particles according to claim 1, wherein said modified polysiloxanes are selected from the group consisting of:

(A) polysiloxanes modified with at least one compound selected from the group consisting of polyethers, polyesters and epoxy compounds, and

(B) polysiloxanes whose molecular terminal is modified with at least one group selected from the group consisting of carboxylic acid groups, alcohol groups and a hydroxyl group.

4. Black magnetic composite particles according to claim 3, wherein said polysiloxanes modified with at least one compound selected from the group consisting of polyethers, polyesters and epoxy compounds are represented by the general formula (III), (IV) or (V):



wherein R<sup>3</sup> is  $-(\text{CH}_2)_h-$ ; R<sup>4</sup> is  $-(\text{CH}_2)_i-\text{CH}_3$ ; R<sup>5</sup> is  $-\text{OH}$ ,  $-\text{COOH}$ ,  $-\text{CH}=\text{CH}_2$ ,  $-\text{C}(\text{CH}_3)=\text{CH}_2$  or  $-(\text{CH}_2)_j-\text{CH}_3$ ; R<sup>6</sup> is  $-(\text{CH}_2)_k-\text{CH}_3$ ; g and h are each integers of 1 to 15; i, j and k are each integers of 0 to 15; e is an integer of 1 to 50; and f is an integer of 1 to 300;



wherein R<sup>7</sup>, R<sup>8</sup> and R<sup>9</sup> are  $-(\text{CH}_2)_q-$  which may be the same or different; R<sup>10</sup> is  $-\text{OH}$ ,  $-\text{COOH}$ ,  $-\text{CH}=\text{CH}_2$ ,  $-\text{C}(\text{CH}_3)=\text{CH}_2$  or  $-(\text{CH}_2)_r-\text{CH}^3$ ; R<sup>11</sup> is  $-(\text{CH}_2)_s-\text{CH}_3$ ; n and q are each integers of 1 to 15; r and s are each integers of 0 to 15; e' is an integer of 1 to 50; and f is an integer of 1 to 300; or

56



wherein R<sup>12</sup> is  $-(\text{CH}_2)_v-$ ; v is an integer of 1 to 15; t is an integer of 1 to 50; and u is an integer of 1 to 300.

5. Black magnetic composite particles according to claim 3, wherein said polysiloxanes whose molecular terminal is modified with at least one group selected from the group consisting of carboxylic acid groups, alcohol groups and a hydroxyl group are represented by the general formula (VI):



wherein R<sup>13</sup> and R<sup>14</sup> are  $-\text{OH}$ ,  $\text{R}^{16}\text{OH}$  or  $\text{R}^{17}\text{COOH}$  which may be the same or different; R<sup>15</sup> is  $-\text{CH}_3$  or  $-\text{C}_6\text{H}_5$ ; R<sup>16</sup> and R<sup>17</sup> are  $-(\text{CH}_2)_y-$ ; y is an integer of 1 to 15; w is an integer of 1 to 200; and x is an integer of 0 to 100.

6. Black magnetic composite particles according to claim 1, wherein said alkoxysilane compound is represented by the general formula (I):



wherein R<sup>1</sup> is  $\text{C}_6\text{H}_5-$ ,  $(\text{CH}_3)_2\text{CHCH}_2-$  or  $\text{n-C}_b\text{H}_{2b+1}-$  where b is an integer of 1 to 18; X is  $\text{CH}_3\text{O}-$  or  $\text{C}_2\text{H}_5\text{O}-$ ; and a is an integer of 0 to 3.

7. Black magnetic composite particles according to claim 6, wherein said alkoxysilane compound is methyl triethoxysilane, dimethyl diethoxysilane, phenyl triethoxysilane, diphenyldiethoxysilane, methyltrimethoxysilane, dimethyldimethoxysilane, phenyltrimethoxysilane, diphenyldiethoxysilane, isobutyltrimethoxysilane or decyltrimethoxysilane.

8. Black magnetic composite particles according to claim 1, wherein said polysiloxanes are represented by the general formula (II):



55 wherein R<sup>2</sup> is  $\text{H}-$  or  $\text{CH}_3-$ , and d is an integer of 15 to 450.

9. Black magnetic composite particles according to claim 8, wherein said polysiloxanes are ones having methyl hydrogen siloxane units.

60 10. Black magnetic composite particles according to claim 1, wherein said fluoroalkylsilane compounds are represented by the general formula (VII):



65 wherein R<sup>18</sup> is  $\text{CH}_3-$ ,  $\text{C}_2\text{H}_5-$ ,  $\text{CH}_3\text{O}-$  or  $\text{C}_2\text{H}_5\text{O}-$ ; X is  $\text{CH}_3\text{O}-$  or  $\text{C}_2\text{H}_5\text{O}-$ ; and z is an integer of 0 to 15; and a' is an integer of 0 to 3.

11. Black magnetic composite particles according to claim 1, wherein the amount of said coating organosilicon compounds is 0.02 to 5.0% by weight, calculated as Si, based on the total weight of the organosilicon compounds and said magnetic iron oxide particles.

12. Black magnetic composite particles according to claim 1, wherein said carbon black coat is obtained by mixing carbon black fine particles having a particle size of 0.002 to 0.05  $\mu\text{m}$  with the magnetic iron oxide particles coated with at least one organosilicon compound while applying a shear force.

13. Black magnetic composite particles according to claim 1, wherein the thickness of said carbon black coat is not more than 0.04  $\mu\text{m}$ .

14. Black magnetic composite particles according to claim 1, wherein said black magnetic composite particles have an average particle diameter of 0.06 to 1.0  $\mu\text{m}$ .

15. Black magnetic composite particles according to claim 1, wherein said black magnetic composite particles have a geometrical standard deviation of particle sizes of 1.01 to 2.0.

16. Black magnetic composite particles according to claim 1, wherein said black magnetic composite particles have a BET specific surface area value of 1 to 200  $\text{m}^2/\text{g}$ , a flowability index of 45 to 80 and a blackness (L\* value) of 15 to 20.

\* \* \* \* \*